

# United States Patent [19]

Kondo et al.

[11] Patent Number: 4,460,648

[45] Date of Patent: Jul. 17, 1984

[54] POROUS BICOMPONENT ACRYLIC SYNTHETIC FIBERS COMPRISING CELLULOSE ACETATE IN AN ACRYLIC MATRIX AND METHOD FOR PRODUCING SAID FIBERS

[75] Inventors: Yoshikazu Kondo; Toshihiro Yamamoto; Takaji Yamamoto, all of Hofu, Japan

[73] Assignees: Kanebo, Ltd., Tokyo; Kanebo Synthetic Fibers Ltd., Osaka, both of Japan

[21] Appl. No.: 397,280

[22] Filed: Jul. 12, 1982

## Related U.S. Application Data

[62] Division of Ser. No. 156,993, Jun. 6, 1980, Pat. No. 4,351,879.

## Foreign Application Priority Data

Jun. 18, 1979 [JP] Japan ..... 55-77046  
Jun. 18, 1979 [JP] Japan ..... 55-77049  
Oct. 1, 1979 [JP] Japan ..... 55-127065  
Oct. 1, 1979 [JP] Japan ..... 55-127066

[51] Int. Cl.<sup>3</sup> ..... B32B 27/02; D01F 8/10;  
D02G 3/00

[52] U.S. Cl. ..... 428/373; 264/176 F;  
264/177 F; 264/182; 428/370; 428/374;  
428/376; 428/398; 428/400

[58] Field of Search ..... 264/176 F, 177 F, 182;  
428/373, 374, 376, 398, 400

## References Cited

### U.S. PATENT DOCUMENTS

4,351,879 9/1982 Kondo et al. ..... 428/376

### FOREIGN PATENT DOCUMENTS

39-14029 7/1964 Japan .  
39-14030 7/1964 Japan .  
42-6014 3/1967 Japan .

43-551 1/1968 Japan .  
44-11969 5/1969 Japan .

## OTHER PUBLICATIONS

Chemical Abstract, 78:148816, (1973).  
Chemical Abstract, 89:130849, (1978).  
Chemical Abstract, 91:158915, (1979).  
Chemical Abstract, 92:23676, (1980).  
Chemical Abstract, 94:4881, (1981).

Primary Examiner—James C. Cannon  
Attorney, Agent, or Firm—Flynn, Thiel, Boutell & Tanis

[57]

## ABSTRACT

Porous acrylic synthetic fibers having water absorption property and having substantially no microvoids but having mainly macrovoids are produced by spinning an organic solvent solution containing 15~35% by weight of a polymer consisting of 2~30 parts by weight of cellulose acetate and 70~98 parts by weight of an acrylic polymer into a coagulation bath at a temperature of no higher than 30° C., primarily drawing the spun fibers at a draw ratio of 2.5~8.0 times to form water swelled fibers wherein macrovoids are distributed, drying the water swelled fibers at a temperature of 100°~180° C. to a water content of no greater than 1.0% by weight and secondarily drawing the dried fibers under wet heat to elongate the macrovoid structure.

This invention includes acrylic composite fibers having water absorption property wherein at least one of components A and B consisting of 2~50% by weight of cellulose acetate and 50~98% by weight of an acrylic polymer and another component B consisting of an acrylic polymer are bonded in a conjugate ratio of 2/8~8/2 (by weight) along the fiber axial direction, one component A has substantially no microvoid but has mainly macrovoids, and the method for producing said acrylic composite fibers.

8 Claims, 8 Drawing Figures



FIG. 1



FIG. 2



FIG.3



FIG.4



FIG.5



FIG.6



FIG. 7



FIG. 8



**POROUS BICOMPONENT ACRYLIC SYNTHETIC FIBERS COMPRISING CELLULOSE ACETATE IN AN ACRYLIC MATRIX AND METHOD FOR PRODUCING SAID FIBERS**

This is a division of application Ser. No. 156,993 filed June 6, 1980, now U.S. Pat. No. 4,351,879.

The present invention relates to porous acrylic synthetic fibers and acrylic composite fibers having a water absorption property and methods for producing these fibers.

Natural fibers, such as cottons, wools, silks and others have a water absorption property of 20-40% and absorb perspiration satisfactorily so that a pleasant feeling is obtained during wearing, but synthetic fibers are low in the antistatic property and the hygroscopicity and have no water absorption property and perspiration absorption property and therefore the synthetic fibers are inferior to natural fibers in the commercial value. Particularly, if underwears, stockings, blankets, sports wears, etc. have no water- and perspiration-absorption property, the perspiration condenses on the fiber surface and such fibers are sticky and cause a cold feeling and are poor in regulation of the body temperature and an unpleasant feeling when wearing can not be avoided.

For improving the water- and perspiration-absorption property of synthetic fibers, various improvements have been heretofore proposed. The major parts of the improvements consist in the formation of microvoids in the fibers or the formation of unevenness on the fiber surface. For example, Japanese Patent Laid Open Application No. 25,418/72, Japanese Patent Nos. 665,549 and 702,476 and Japanese Patent Application Publication No. 6,650/73 have disclosed processes for producing porous acrylic fibers by selecting such a mild drying condition that microvoids remain in the swelled gel tow during the production of acrylic fibers. Furthermore, Japanese Patent Laid Open Application No. 25,416/72, Japanese Patent Application Publication Nos. 8,285/73 and 8,286/73 have disclosed that a water soluble compound is incorporated in the swelled gel tow during the production of acrylic fibers and the swelled gel tow is dried and after-treated, after which the water soluble compound is dissolved off to reform the voids. The common concept in the above described processes consists in that microvoids inherently formed during the production of the acrylic fibers are maintained in the final product to obtain porous acrylic fibers. The microvoids formed in the swelled gel tow are very thermally unstable. Therefore, it is impossible to effect treatment at a high temperature in the steps for producing the fibers, particularly at the drying, shrinking and crimp setting steps and the heat resistance, form stability and crimp stability of the final product are poor and the commercial value of the product is considerably deteriorated. The radius of the voids in the obtained product is very small, such as 10-1,000 Å. Since numerous microvoids are uniformly distributed in the fibers, the strength and elongation of the fibers are low, the luster is poor and the dyed color is not clear. Furthermore, since numerous microvoids are uniformly distributed, the heat resistance of the fibers is low and in a high temperature dyeing, steaming treatment, pressing treatment and the like, the voids are eliminated, the water absorption property is deteriorated, the color tone is varied, the form stability is deteriorated and the qualities are degraded.

When it is attempted to develop the water absorption property by these voids, the microvoids are apt to be formed as closed voids and they hardly form passages through which water is absorbed into the fibers and this proposal is not effective. In order to obtain a certain degree of water absorption property, a fairly large number of microvoids are necessary and this further deteriorates the fiber properties and commercial value. It has been previously attempted to improve the feel and the dyeability by mix-spinning of cellulose acetate-acrylic polymer or cellulose acetate-modacrylic copolymer. For example, Japanese Patent Nos. 222,873 and 243,556 and Japanese Patent Application Publication No. 14,029/64 have disclosed that the spinning solution obtained by mixing cellulose acetate with acrylic polymer or modacrylic copolymer is spun to obtain fibers having improved dyeability and feel. The fibers obtained in these processes are dense and have no water absorption property due to voids in the fiber interior. In addition, Japanese Patent No. 433,941 has disclosed that cellulose acetate is added during polymerization of the acrylic polymer as a means for mixing cellulose acetate, but when the polymer obtained by mixing cellulose acetate during polymerization of the acrylic polymer is used, the heat resistance of the spun fibers is deteriorated owing to the degradation of cellulose acetate and troubles occur during the steps for producing the fibers and the product having the satisfactory quality can not be obtained. Japanese Patent No. 556,549 and Japanese Patent Laid Open Application Nos. 118,027/75 and 118,026/75 have described that cellulose acetate or a mixture of cellulose acetate and titanium oxide and the like is finely distributed in acrylic polymer or modacrylic polymer to obtain animal hair-like fibers but it can not provide porous fibers having a high water absorption property as is obtained in the present invention. German Patent Laid Open Application No. 2,901,778 has proposed acrylic fibers having a water absorption property, consisting of a porous core portion having a large number of microvoids and macrovoids and a skin portion having a high density, but these fibers have a large number of microvoids, so that the yarn property and dyeability are deteriorated. Further it is not easy to produce fibers having uniform microvoids and it is difficult to obtain fibers having stable quality. Fibers having excellent yarn property, heat resistance, dyeability and water absorption property as in the present invention can not be obtained by this procedure.

From the above described reasons porous acrylic synthetic fibers having improved water absorption property, heat resistance, dyeability and luster can not be obtained by the prior processes.

Japanese Patent Application Publication No. 6,014/67 has disclosed acrylic composite fibers obtained by conjugate spinning acrylic polymers having different contents of ionic hydrophilic groups in which as a composite component having a smaller amount of said hydrophilic group, use is made of an acrylic polymer containing a cellulosic polymer which is obtained by solution polymerization of acrylic monomer in the presence of a cellulosic polymer soluble in a solvent for polymerization of the acrylic polymer. Japanese Patent No. 520,657 has disclosed that in the conjugate spinning of acrylonitrile polymer containing an acidic group and acrylonitrile polymer containing a basic group, a cellulosic polymer is contained in a component having a lower shrinkage among these polymers. However, these processes aim to improve the crimpability and

dyeability and to provide the resilient feeling of the cellulosic polymer but do not aim at porous acrylic composite fibers having a water absorption property and these fibers can not be obtained by these processes. The inventors have diligently studied to obviate the prior defects and accomplished the present invention.

An object of the present invention is to provide porous acrylic synthetic fibers and acrylic composite fibers having excellent water absorption property and good yarn properties.

Another object of the present invention is to provide methods for producing porous acrylic synthetic fibers and acrylic composite fibers having excellent water absorption property and good yarn properties commercially easily and cheaply.

The present invention consists in porous acrylic synthetic fibers having substantially no microvoids but having mainly macrovoids, which consist of 2~30% by weight of cellulose acetate and 70~98% by weight of an acrylic polymer and have a surface area A of voids of no greater than 15 m<sup>2</sup>/g and a porosity V of 0.50~0.75 cm<sup>3</sup>/g, V/A being 1/30 or more.

The process of the present invention comprises spinning an organic solvent solution containing 15~35% by weight of a polymer consisting of 2~30 parts by weight of cellulose acetate and 70~98 parts by weight of an acrylic polymer into a coagulation bath at a temperature of no higher than 30° C. to obtain fibers wherein the formation of microvoids is restrained, effecting primary drawing of the spun fibers at a draw ratio of 2.5~8 times, drying the fibers in a water swelled state having distributed macrovoids at a temperature of 100°~180° C. to a water content of no greater than 1.0% by weight to substantially eliminate microvoids and effecting secondary drawing of the dried fibers under wet heat at a draw ratio of no greater than 3 times to promote the macrovoid structure.

Furthermore, the present invention relates to acrylic composite fibers and a method for producing said fibers, which is discussed later.

The acrylic synthetic fibers according to the present invention consist of 2~30% by weight, preferably 3~25% by weight, more preferably 6~20% by weight, more particularly from more than 10% by weight to 18% by weight of cellulose acetate and 70~98% by weight, preferably 75~97% by weight, more preferably 80~94% by weight, more particularly from 82% by weight to less than 90% by weight of an acrylic polymer. When the amount of cellulose acetate distributed in the fibers is less than 2% by weight, phase separation thereof from the acrylic polymer is insufficient and the satisfactory water absorption property can not be obtained, while when said amount exceeds 30% by weight, the phase separation becomes excessive and the strength and elongation, dyeability and luster of the fibers are deteriorated, so that these amounts should be avoided.

Cellulose acetate to be used in the present invention is not particularly limited but in general, is one having a combined acetic acid of 48~63% and an average polymerization degree of 50~300.

The acrylic polymers to be used in the present invention contain at least 80% by weight, preferably 85~93% by weight of acrylonitrile and may contain less than 20% by weight of copolymerizable monomers, for example alkyl acrylates, or methacrylates, such as methyl acrylate, methyl methacrylate, ethyl acrylate, amides, such as acrylamide, methacrylamide, N-mono-

substituted or N,N-disubstituted amides thereof, vinyl acetate, sulfonic acid group-containing monomers, such as styrenesulfonic acid, allylsulfonic acid, methallylsulfonic acid and the salts thereof. In particular, when 5 0.3~1.5% by weight, preferably 0.5~1.2% by weight of allylsulfonic acid or methallylsulfonic acid or the salts thereof is copolymerized, the dyeability is not only improved, but also the formation of numerous microvoids is prevented, whereby the degradation of the 10 heat resistance is prevented and porous fibers having macrovoids and excellent water absorption property can be obtained.

The acrylic polymer of the acrylic synthetic fibers according to the present invention may contain an 15 acrylic copolymer containing 5~30% by weight of a monomer having the general formula



wherein X is R<sub>2</sub> or



R<sub>1</sub> and R<sub>3</sub> are H or CH<sub>3</sub>, R<sub>2</sub> is H, NH<sub>4</sub> or an alkali metal, and 1 and m are an integer of 0~50 and 0<1+m≤50, and the acrylic copolymer is no greater than about 33% by weight based on the total polymer composing the acrylic synthetic fibers. By incorporating the above described acrylic copolymer in the acrylic synthetic fibers, the dispersability of cellulose acetate is improved. As the monomers to be copolymerized in the acrylic copolymers shown by the above described general formula, acrylic acid, methacrylic acid and



are preferable in view of the polymerizability, discoloration and resistance to water solubility. As the length of the ethylene glycol chain or the propylene glycol chain contained in these monomers is larger, the hydrophilic property of the acrylic copolymer is increased and the content is permitted to be smaller, but when 1+m exceeds 50, the polymerizability and solubility of the acrylic copolymer are degraded. As the monomers copolymerizable in the acrylic copolymer other than the monomers having the above described general formula, the above described monomers to be used in the polymerization of the acrylic polymers may be used. The acrylic copolymer contains at least 70% by weight of acrylonitrile.

The acrylic synthetic fibers according to the present invention have substantially no microvoids but have mainly macrovoids and the macrovoids contribute to the water absorption property. In the acrylic synthetic fibers according to the present invention, cellulose acetate is distributed in an elongated form having the longest dimension parallel to the fiber axis and generally has voids in the circumference and the inner portion of cellulose acetate and the ratio of the length to the diameter of the elongated cellulose acetate is generally 10 or more. The voids present in the distributed elongated cellulose acetate are macrovoids caused by the phase

separation of cellulose acetate and acrylic polymer and are further elongated by the secondary drawing. The acrylic polymer component in the acrylic synthetic fibers of the present invention has substantially the same degree of denseness as usual acrylic synthetic fibers and has substantially no microvoids. The term "substantially no microvoids" used herein means that the ratio (by volume) of microvoids occupied in the porosity (V) of the fibers is not greater than 30%, preferably not greater than 25%, more preferably not greater than 20%, more particularly not greater than 15%. The term "microvoid" used herein means voids having a diameter of less than 2,000 Å.

The water absorption property of the acrylic synthetic fibers according to the present invention can be obtained owing to these macrovoids and the ratio of the macrovoids occupied in the porosity is at least 70%, preferably at least 75%, more preferably at least 80%, more particularly at least 85%. Cellulose acetate is distributed not only in the inner portion of the cross section of the fiber but also in the fiber wall, so that macrovoids are observed at the fiber surface. The high water absorption property of the acrylic synthetic fibers of the present invention is presumably due to the fact that the voids opening at the fiber surface communicate with the macrovoids in the inner portion of the fibers.

Then, the acrylic synthetic fibers according to the present invention will be explained with reference to the accompanying drawings, wherein:

FIG. 1 is an optical photomicrograph (magnification: 200 times) of the cross section of conventional acrylic fibers;

FIG. 2 is an optical photomicrograph (magnification: 200 times) of the cross section of porous acrylic fibers having a water absorption property, which contain cellulose acetate and in which a large number of microvoids are formed together with macrovoids;

FIG. 3 is an optical photomicrograph (magnification: 200 times) of the cross section of porous acrylic fibers of the present invention;

FIGS. 4, 5 and 6 are electron micrographs (magnification: 12,000 times) of the cross sections of the fibers shown in FIGS. 1~3 respectively;

FIG. 7 is an electron micrograph (magnification: 12,000 times) of the cross section of conventional acrylic fiber having microvoids, and

FIG. 8 is an optical photomicrograph (magnification: 200 times) of the cross section of acrylic composite fibers of the present invention wherein an acrylic polymer (component A) containing cellulose acetate and an acrylic polymer (component B) are bonded in side-by-side relation.

In FIG. 2 and FIG. 3, fibers in which red dye stuff was impregnated so that the judgement of the presence of microvoids was made easy, were used as the samples.

As seen from FIG. 1, the usual acrylic fiber does not substantially have voids. In FIG. 2, since macrovoids are observed but the fibers have numerous microvoids, the dye stuff penetrates along the entire cross section of the fibers. In the fibers according to the present invention, as seen from FIG. 3, only macrovoids are observed and microvoids are not substantially observed.

The usual acrylic fiber in FIG. 4 is very dense and no microvoids are observed. FIG. 5 shows apparently that a large number of microvoids are present in the inner portion of the fiber. On the other hand, FIG. 6 shows that the fiber of the present invention has substantially the same density as the usual acrylic fiber at the portion

other than macrovoids. The microvoid structure is apparently observed from FIG. 7 in the conventional acrylic fiber having the microvoid structure.

In the acrylic synthetic fibers of the present invention, the surface area A of voids is no greater than 15 m<sup>2</sup>/g, preferably 0.02~10 m<sup>2</sup>/g, a porosity V is 0.05~0.75 cm<sup>3</sup>/g, preferably 0.05~0.60 cm<sup>3</sup>/g and V/A is 1/30 or more, preferably 1/20 or more.

The surface area A(m<sup>2</sup>/g) of voids in the fibers was determined as follows. Nitrogen gas was adsorbed in the fibers at the temperature of liquid nitrogen, the total surface area of the fibers was determined by the BET equation and from this value was subtracted the surface area of the outer skin of the fibers. The amount of the fibers to be measured was adjusted so that the value of the total surface area to be measured is 1 m<sup>2</sup> or more.

The porosity V(cm<sup>3</sup>/g) was determined as follows. A density  $\rho$ (g/cm<sup>3</sup>) of a film prepared so as to have the same composition as the fiber and a high density, was measured and an average cross sectional area of the fibers containing the voids was determined by photographic process and referred to as S(cm<sup>2</sup>) and an actual average cross sectional area So(cm<sup>2</sup>) of the fibers at the portion containing no voids was determined from the following equation (1) and the porosity V was determined from the following equation (2).

$$So = \frac{De}{900000 \times \rho} \quad (1)$$

De:Denier

$$V = \frac{1}{\rho} \times \frac{S - So}{So} \quad (2)$$

The ratio of microvoids occupied in the porosity was calculated by measuring the microvoid content by means of a mercury porosimeter. Firstly, the fibers are opened and weighed and then filled in a cell of a mercury porosimeter and a pressure and an amount of mercury pressed in are recorded while pressing mercury at room temperature. Between a diameter D(μ) of the voids and a pressure P(psi) necessary for filling mercury in the voids, there is a relation shown by the following formula

$$D = (175/P)$$

By measuring P and the amount of mercury pressed in the diameter D(μ) and the volume (cm<sup>3</sup>/g) of the voids are determined. From these data, a void distribution curve is obtained and an amount of the voids in which D is 0.2μ or less is determined, which is referred to as the microvoid content (cm<sup>3</sup>/g) in 1 g of the fibers.

When the porosity V is less than 0.05 cm<sup>3</sup>/g, the water absorption property is not satisfied, while when the porosity V exceeds 0.75 cm<sup>3</sup>/g, the strength and elongation of the fibers are degraded and the luster and dyeability are adversely affected, so that these values should be avoided.

When the surface area A of the voids exceeds 15 m<sup>2</sup>/g, the microvoids in the fibers increase and the strength and elongation are not only deteriorated but also the dyeability and heat resistance are deteriorated.

When V/A is less than 1/30, the water absorption property is not satisfied or the heat resistance, dyeability and the like as well as the strength and elongation are deteriorated. Furthermore, it has been found from the experi-

mental data of the inventors that when V/A is less than 1/30, the voids in the fibers become small and if the size is calculated into, for example a sphere, the diameter becomes less than 2,000 Å and the excellent water absorption property can not be obtained and the strength and elongation are deteriorated.

The acrylic synthetic fibers according to the present invention are produced by spinning an organic solvent solution containing 15~35% by weight, preferably 17~30% by weight of a polymer consisting of 2~30 parts by weight, preferably 3~25 parts by weight, more preferably 6~20 parts by weight, more particularly from more than 10 parts by weight to 18 parts by weight of cellulose acetate, and 70~98 parts by weight, preferably 75~97 parts by weight, more preferably 80~94 parts by weight, more particularly 82~90 parts by weight of an acrylic polymer or a blend of an acrylic polymer and an acrylic copolymer into a coagulation bath at a temperature of no higher than 30° C. When the amounts of cellulose acetate, an acrylic polymer or a blend of an acrylic polymer and an acrylic copolymer are beyond these range, acrylic synthetic fibers having an excellent water absorption property and yarn properties can not be obtained. When the concentration of the polymer is less than 15% by weight, the production cost becomes higher and the formation of microvoids increases to deteriorate the strength and elongation. While when the concentration exceeds 35% by weight, the viscosity increases, whereby the operability and spinnability are deteriorated and further the yarn properties are degraded, so that these amounts should be avoided.

As the organic solvent to be used in the present invention, mention may be made of common solvents for cellulose acetate, acrylic copolymers and acrylic copolymers but in general, organic solvents, such as dimethylformamide, dimethylacetamide, dimethylsulfoxide, ethylene carbonate and the like are preferable in view of the recovery and purification of the solvents. As the coagulation bath, use may be made of an aqueous solution of an organic solvent, such as dimethylformamide, dimethylacetamide, dimethylsulfoxide, ethylene carbonate and the like, and organic solvents, such as propyl alcohol, kerosene and the like, but an aqueous solution of an organic solvent to be used for dissolving the polymer is particularly preferable.

The process for mixing cellulose acetate and an acrylic polymer or mixing an acrylic copolymer to said mixture is not particularly limited. For example, each of the polymers is dissolved in a common solvent and the obtained solution are mixed or these polymers are concurrently added and dissolved in a common solvent.

Water may be added to the spinning solution within the range which does not cause gelation of the spinning solution. This addition of water is effective for controlling the viscosity of the spinning solution and preventing the formation of microvoids in the spun fibers. Interestingly, the inventors have found that the dispersed state of the elongated cellulose acetate in the spun fibers varies depending upon the water content in the spinning solution. Namely, when the water content in the spinning solution is increased, the dispersed state of the elongated cellulose acetate becomes longer, and conversely as the water content decreases, the form becomes spherical. A similar result is obtained depending upon the variation of the viscosity of the spinning solution.

The spinning can be carried out under the same conditions as are employed for preparing conventional acrylic synthetic fibers except that the temperature of the coagulation bath cannot be higher than 30° C. Several stages of spinning baths are used and the primary drawing and water washing are carried out. The primary draw ratio is 2.5~8 times, preferably 3~6 times. When the primary draw ratio is less than 2.5 times, the drawing and orientation of the fibers are insufficient and therefore the strength is low and cracks are formed in the fibers and such a drawing should be avoided. While, when the draw ratio exceeds 8 times, the densification excessively proceeds and a satisfactory water absorption property can not be obtained and the operability is deteriorated, so that such draw ratios should be avoided.

The spinning draft ratio may be the usual condition, but for restraining the formation of microvoids a lower draft ratio is preferable. The temperature of the coagulation bath for restraining the formation of microvoids must be not higher than 30° C., preferably not higher than 25° C., more preferably not higher than 20° C. When the temperature of the coagulation bath is higher than 30° C., a large number of microvoids are formed and the yarn properties and quantity of the obtained fibers are considerably deteriorated.

In the primary drawn fibers, the dispersion of the elongated cellulose acetate, and the voids formed by the phase separation of cellulose acetate and the acrylic polymer become more distinct. But the fibers contain a large number of microvoids inherently contained in the usual swelled gel tow. These microvoids are not desirable because of the deterioration of the heat resistance, dyeability and luster of the fibers. Hence, the fibers wherein the microvoids and macrovoids coexist, are dried to eliminate the microvoids but, in this case, the drying is carried out at a temperature of 100°~180° C., preferably 105°~150° C. until the water content becomes no greater than 1.0% by weight, whereby only the microvoids are eliminated and the macrovoids formed due to the phase separation are maintained. When the drying temperature is lower than 100° C., the microvoids formed in the acrylic polymer can not be completely collapsed by drying and the strength and elongation, luster, dyeability and heat resistance of the fibers are deteriorated. While when the drying temperature exceeds 180° C., the fibers are hardened and discolored, so that such a temperature should be avoided. For drying, it is desirable for eliminating the microvoids to

use a hot roller type dryer in which the fibers are brought into contact with a metal surface heated at a high temperature. In addition, if the drying is effected by blowing hot air at a temperature of 120°~170° C. as a supplemental means, the drying can be effected more uniformly, so that such a means is desirable. The water content of the dried fibers must be no greater than 1.0%. When the water content exceeds 1.0%, the uneven drying of the fibers occurs and a large number of microvoids partially remain resulting in unevenness of dyeing, luster, and strength of the fibers and the uniformity of equality is deteriorated. In this drying step, a torque motor may be used to effect shrinkage of 5~15% together with the drying.

The dried fibers should be subjected to a secondary drawing under wet heat to a draw ratio of no greater than 3 times, preferably 1.05~2 times in order to make the phase separation of the acrylic polymer and cellulose acetate in the fibers more distinct and to promote

the macrovoid structure and improve the water absorption property and provide moderate physical properties of the fiber. The secondary drawing includes stretching shrinkage of substantial draw ratio of no greater than 1.0. But in order to elongate the macrovoid structure, the draw ratio is preferred to be at least 1.05, particularly at least 1.1. When the draw ratio exceeds 3 times, yarn breakage occurs and if the temperature is raised in order to prevent yarn breakage, the stickiness of the fibers occurs and the water absorption property is considerably deteriorated. After the secondary drawing, the fibers are subjected to after-treating steps for imparting good spinnability and performance to the fibers, such as wet heat shrinking step, oiling step, crimping step and crimp-setting step to obtain the final product.

Now, an explanation will be made with respect to acrylic composite fibers according to the present invention. The composite fibers according to the present invention are ones having a water absorption property obtained by bonding a component A consisting of 2~50% by weight of cellulose acetate and 50~98% by weight of an acrylic polymer and a component B consisting of an acrylic polymer in a weight ratio of 2/8~8/2 along the fiber axial direction, the component A having substantially no microvoids but having mainly macrovoids, and having a porosity of the entire fibers of 0.05~0.75 cm<sup>3</sup>/g and a surface area of voids of no greater than 15 m<sup>2</sup>/g. or ones having a water absorption property and latent crimpability obtained by eccentrically bonding two components A and B consisting of 2~50% by weight of cellulose acetate and 50~98% by weight of an acrylic polymer, a plasticizing component in the acrylic polymer in both the components A and B having a difference of at least 2% by weight, in a weight ratio of 7/3~3/7, a total amount of cellulose acetate in the fibers being 2~30% by weight, having substantially no microvoids but having macrovoids, and having a porosity of 0.05~0.75 cm<sup>3</sup>/g and a surface area of voids of no greater than 15 m<sup>2</sup>/g.

The process for producing the composite fibers according to the present invention comprises conjugate spinning two organic solvent solutions A and B in which at least one solution contains a polymer consisting of 2~50% by weight of cellulose acetate and 50~98% by weight of an acrylic polymer, into a coagulation bath at a temperature of no higher than 30°C. through common spinning orifices to form composite fibers in which the formation of microvoids is restrained effecting primary drawing of the spun fibers in a draw ratio of 2.5~8 times, drying the water swelled fibers containing distributed macrovoids at a temperature of 100°~180° C. to a water content of no greater than 1.0% by weight to substantially eliminate microvoids and then effecting secondary drawing of the dried fibers in a draw ratio of no greater than 3 times under wet heat to promote the macrovoid structure.

In the case of acrylic composite fibers in which only the component A contains cellulose acetate, when an amount of a plasticizing component in acrylic polymers composing the components A and B, such as methyl acrylate, methyl methacrylate, ethyl acrylate, ethyl methacrylate, acrylamide, vinyl acetate, 2-hydroxyethyl acrylate, 2-hydroxyethyl methacrylate and the like is different in an amount of at least 2% by weight and the component A and the component B are conjugate spun eccentrically, composite fibers having latent crimpability can be obtained. On the other hand, when there is substantially no difference in the content of the

above described plasticizing component in the acrylic polymers to composing the component A and the component B or both the components are concentrically conjugate spun, composite fibers having substantially no latent crimpability can be obtained.

The component A and the component B are bonded in a conjugate ratio of 2/8~8/2, preferably 3/7~7/3, more preferably 4/6~6/4. If the component A is smaller than 2/8 in the conjugate ratio, a satisfactory water absorption property can not be given to the composite fibers, while if the component A exceeds 8/2, the luster and color brightness after dyeing are deteriorated. As the plasticizing components in both the components A and B to be used in the acrylic composite fibers containing cellulose acetate, mention may be made of the above described compounds. The difference of the content of the plasticizing component in both the components is at least 2% by weight, preferably 2.5~5% by weight. The components A and B are bonded eccentrically, preferably in side-by-side relation.

When the difference of the content of the above described plasticizing component is less than 2% by weight, it is impossible to obtain composite fibers having substantial latent crimpability. The component A and the component B are bonded in a conjugate ratio of 3/7~7/3, preferably 4/6~6/4. When the ratio exceeds this range, composite fibers having excellent crimpability can not be obtained. The conjugate ratio of the acrylic composite fibers according to the present invention can be conveniently varied by varying the extruded amount of the solutions of the components A and B in an organic solvent or the polymer concentration.

When the component A or both the components A and B contain cellulose acetate, the amount of cellulose acetate is 2~50% by weight, preferably 3~40% by weight, more preferably 5~30% by weight. When the amount of cellulose acetate distributed in the component A or both the components A and B is less than 2% by weight, the phase separation of the acrylic polymer is insufficient and the water absorption property can not be satisfied, while when said amount exceeds 50% by weight, the strength and elongation in the component A or both the components A and B become considerably lower and both the components are disengaged, so that these amounts should be avoided.

When cellulose acetate is contained in both the components A and B, the total amount of cellulose acetate contained in both the components A and B is 2~30% by weight, preferably 2~25% by weight, more preferably 3~20% by weight. When the total amount is less than 2% by weight, the water absorption property is not satisfied and when said amount exceeds 30% by weight, the yarn properties, such as strength and elongation of the composite fibers are deteriorated and these amounts should be avoided.

Concerning the acrylic polymers, acrylic copolymers and cellulose acetate to be used for the acrylic composite fibers according to the present invention, the above described explanation concerning the acrylic synthetic fibers can be applied.

Cellulose acetate in at least one component of the composite fibers of the present invention is distributed in an elongated form parallel to the fiber axis, and generally has voids around the elongated cellulose acetate and in the inner portion and the ratio of the length of the distributed elongated cellulose acetate to the diameter thereof is usually 10 or more.

The component containing cellulose acetate in the composite fibers of the present invention does not substantially have microvoids but has mainly macrovoids and these macrovoids contribute to the water absorption property.

FIG. 8 is an optical photomicrograph (magnification: 200 times) of the cross section of the acrylic composite fibers of the present invention in which the component A (acrylic polymer containing cellulose acetate) and the component B (acrylic polymer) are bonded in side-by-side relation and it can be seen from FIG. 8 that macrovoids are observed in the component A and the component B is dense.

The acrylic composite fibers of the present invention have a porosity of  $0.05 \sim 0.75 \text{ cm}^3/\text{g}$ , preferably  $0.05 \sim 0.60 \text{ cm}^3/\text{g}$  and a surface area of voids of no greater than  $15 \text{ m}^2/\text{g}$ , preferably  $0.02 \sim 10 \text{ m}^2/\text{g}$  as the entire fibers.

When the porosity is less than  $0.05 \text{ cm}^3/\text{g}$ , the water absorption property is not satisfactory, while when the porosity exceeds  $0.75 \text{ cm}^3/\text{g}$ , the strength and elongation of the fibers not only are deteriorated, but also the luster and dyeability are adversely affected.

When the surface area of the voids exceeds  $15 \text{ m}^2/\text{g}$ , microvoids increase in the fibers and the strength and elongation decrease and the dyeability and heat resistance are deteriorated.

The organic solvent, coagulation bath condition, and spinning and drawing conditions in the production of the acrylic composite fibers are similar to those in the above described production of acrylic synthetic fibers.

After the secondary drawing, the composite fibers having the latent crimpability may be subjected to after-treatments, such as shrinking-drawing-shrinking in order to enhance the crimpability. After the secondary drawing, the fibers are subjected to after-treatments for giving high spinnability and properties, such as shrinking under wet heat, oiling, crimping, crimp setting and the like, to obtain the final product.

The composite fibers of the present invention can easily develop crimps through hot water treatment and steam treatment.

The porous acrylic synthetic fibers and the acrylic composite fibers according to the present invention can be produced by using not only an organic solvent but also an inorganic solvent, such as aqueous solution of zinc chloride and the like.

The porous acrylic synthetic fibers obtained by the present invention have a high water absorption property and water absorbing rate and are excellent in strength and elongation under wet swelling when absorbing water, and have good luster and brightness when dyed. The acrylic composite fibers of the present invention have a high water absorption property, water

absorbing rate, excellent strength and elongation when absorbing water, good dyeability and unique bulkiness and rich feeling of the inherent composite fibers.

In the natural fibers, the bulkiness and resilient feeling are lost upon wet swelling but in the acrylic synthetic fibers and acrylic composite fibers according to the present invention, the water absorption is a physical mechanism in which water is absorbed in voids in the fibers, so that these fibers are not deteriorated in the bulkiness and resilient feeling and the water absorption property, water- and moisture-permeability are excellent. In addition, acrylic synthetic fibers and composite fibers according to the present invention have a porosity of  $0.05 \sim 0.75 \text{ cm}^3/\text{g}$  and are light in weight and very high in the heat retaining property.

The acrylic synthetic fibers and composite fibers of the present invention, which have such many excellent properties, are optimum for general clothings, sports wears, bedding, curtains, interior and the like. Furthermore, these fibers are satisfactorily used in the field where cotton has been used, as cotton substitutes.

The following examples are given for the purpose of illustration of this invention and are not intended as limitations thereof. In the examples, parts and % mean parts by weight and % by weight unless otherwise indicated. The water absorption of fibers was measured according to DIN-53814, and the crimp property thereof was measured according to JIS L-1074.

#### EXAMPLE 1

A dimethyl formamide (hereinafter abbreviated as DMF) solution containing 21% of a polymer mixture consisting of an acrylic polymer and cellulose acetate in a mixing ratio shown in the following Table 1 was extruded from a spinneret into a coagulation bath consisting of 65% of DMF and 35% of water and kept at 20° C. The acrylic polymer had a composition of acrylonitrile (hereinafter abbreviated as AN): methyl acrylate (hereinafter abbreviated as MA): sodium methylallylsulfonate (hereinafter abbreviated as SMAS) = 90.5:9.0:0.5(%). The extruded filaments were subjected to a primary drawing to draw the filaments to 5 times their original length, and then dried by means of a hot roller type drier kept at 120° C. until the water content of the filaments was decreased to 0.5%. The dried filaments were subjected to a secondary drawing at 100° C. under wet heat to draw the filaments to 1.1 times their original length. The drawn filaments were mechanically crimped and the crimps were set to obtain 3-denier fibers. Properties of the resulting fibers are shown in Table 1. It was found that the ratios of microvoids in the fibers of Experiment Nos. 4 and 5 were 11.3% and 14.6%, respectively.

TABLE 1

| Experiment number | Fiber Property          |                           |                                  |      |                      |                |            |                         |
|-------------------|-------------------------|---------------------------|----------------------------------|------|----------------------|----------------|------------|-------------------------|
|                   | Polymer Mixture         |                           | Void area, A (m <sup>2</sup> /g) | V/A  | Water absorption (%) | Strength (g/d) | Dyeability | Remarks                 |
| Experiment number | Acrylic polymer (parts) | Cellulose acetate (parts) |                                  |      |                      |                |            |                         |
| 1                 | 100                     | 0                         | 0.000                            | 0.00 | —                    | 4              | 3.8        | good Comparative sample |
| 2                 | 99                      | 1                         | 0.021                            | 0.57 | 1/27.1               | 4              | 3.8        | " Comparative sample    |
| 3                 | 98                      | 2                         | 0.116                            | 1.62 | 1/14.0               | 15             | 3.8        | " Present invention     |

TABLE 1-continued

| Experiment number | Polymer Mixture         |                           | Void                             |                                     | Fiber Property |                      |                |               |                    |
|-------------------|-------------------------|---------------------------|----------------------------------|-------------------------------------|----------------|----------------------|----------------|---------------|--------------------|
|                   | Acrylic polymer (parts) | Cellulose acetate (parts) | Porosity, V (cm <sup>3</sup> /g) | Surface area, A (m <sup>2</sup> /g) | V/A            | Water absorption (%) | Strength (g/d) | Dyeability    | Remarks            |
| 4                 | 95                      | 5                         | 0.221                            | 1.70                                | 1<br>7.7       | 25                   | 3.6            | "             | Present invention  |
| 5                 | 90                      | 10                        | 0.357                            | 2.04                                | 1<br>5.7       | 38                   | 3.2            | "             | Present invention  |
| 6                 | 80                      | 20                        | 0.46                             | 2.35                                | 1<br>5.7       | 48                   | 2.6            | somewhat poor | Present invention  |
| 7                 | 70                      | 30                        | 0.588                            | 2.76                                | 1<br>4.7       | 60                   | 1.7            | somewhat poor | Present invention  |
| 8                 | 65                      | 35                        | 0.798                            | 3.09                                | 1<br>3.7       | 80                   | 1.1            | poor          | Comparative sample |
| 9                 | 60                      | 40                        | 1.08                             | 3.09                                | 1<br>2.9       | 100                  | 0.8            | "             | Comparative sample |

## EXAMPLE 2

The same acrylic polymer as used in Example 1 was used, and 3-denier fibers shown in the following Table 2<sup>25</sup> were produced by changing the composition of the

polymer mixture, the extruding condition, the drawing condition, the drying condition and other production conditions. Properties of the resulting fibers are shown in Table 2.

TABLE 2

| Experiment number | Void                             |                                     | Fiber Property |                      |                                           |                    |
|-------------------|----------------------------------|-------------------------------------|----------------|----------------------|-------------------------------------------|--------------------|
|                   | Porosity, V (cm <sup>3</sup> /g) | Surface area, A (m <sup>2</sup> /g) | V/A            | Water absorption (%) | Others                                    | Remarks            |
| 10                | 0.03                             | 0.71                                | 1<br>23        | 5                    | poor in heat resistance and in dyeability | Comparative sample |
| 11                | 0.05                             | 1.82                                | 1<br>36        | 9                    | poor in heat resistance and in dyeability | Comparative sample |
| 12                | 0.10                             | 0.44                                | 1<br>4.4       | 14                   |                                           | Present invention  |
| 13                | 0.35                             | 2.11                                | 1<br>6.0       | 37                   |                                           | Present invention  |
| 14                | 0.75                             | 17.3                                | 1<br>23        | 70                   | low strength and poor dyeability          | Comparative sample |
| 15                | 0.90                             | 25.1                                | 1<br>28        | 87                   | low strength and poor dyeability          | Comparative sample |
| 16                | 1.05                             | 9.83                                | 1<br>9.4       | 104                  | low strength and poor dyeability          | Comparative sample |
| 17                | 0.43                             | 0.94                                | 1<br>2.2       | 45                   | low strength and poor dyeability          | Present invention  |
| 18                | 0.59                             | 0.78                                | 1<br>1.3       | 60                   |                                           | Present invention  |
| 19                | 0.30                             | 13.8                                | 1<br>46        | 33                   | poor in heat resistance and in dyeability | Comparative sample |
| 20                | 0.61                             | 16.8                                | 1<br>27        | 63                   | low strength and poor dyeability          | Comparative sample |
| 21                | 0.51                             | 19.1                                | 1<br>37        | 50                   | low strength and poor dyeability          | Comparative sample |
| 22                | 0.80                             | 26.9                                | 1<br>33        | 76                   | poor in heat resistance and in dyeability | Comparative sample |
| 23                | 0.72                             | 0.95                                | 1<br>1.3       | 73                   |                                           | Present invention  |
| 24                | 0.63                             | 3.21                                | 1<br>5.1       | 64                   |                                           | Present invention  |

## EXAMPLE 3

A polymer mixture consisting of 80 parts of an acrylic polymer, which had a composition of AN:MA:sodium allylsulfonate (hereinafter abbreviated as SAS)=90.2:9.0:0.8(%), and 20 parts of cellulose acetate was dissolved in a solvent shown in the following Table 3 to prepare spinning solutions having a property shown in Table 3. The extrusion of the spinning solution and the after-treatment of the extruded filaments were carried out under the same conditions as described in

Example 1 to obtain 3-denier fibers. However, as the coagulation bath, an aqueous solution containing the same solvent as that used in the spinning solution was used.

Properties of the fibers are shown in Table 3.

In Table 3, the viscosity of the spinning solution was measured at 50° C. by means of a Brookfield viscometer. The stability of the spinning solution was estimated by the stability against gellation at 50° C. and by the stability of dispersion of the acrylic polymer and cellulose acetate in the spinning solution.

TABLE 3

| Experiment number | Solvent            | Spinning Solution                                  |                      |               | Fiber Property                         |                                           |           |                        |             |               |
|-------------------|--------------------|----------------------------------------------------|----------------------|---------------|----------------------------------------|-------------------------------------------|-----------|------------------------|-------------|---------------|
|                   |                    | Concen-<br>tration of<br>polymer<br>mixture<br>(%) | Viscosity<br>(poise) | Stability     | Void                                   |                                           | Water     |                        | Operability | Remarks       |
|                   |                    |                                                    |                      |               | Porosity,<br>V<br>(cm <sup>3</sup> /g) | Surface<br>area, A<br>(m <sup>2</sup> /g) | V/A       | absorp-<br>tion<br>(%) |             |               |
| 25                | Dimethyl acetamide | 10                                                 | 8.5                  | good          | 0.57                                   | 17.9                                      | 1<br>31.4 | 58                     | 1.8         | somewhat poor |
| 26                | Dimethyl acetamide | 15                                                 | 15                   | "             | 0.51                                   | 3.14                                      | 1<br>6.2  | 53                     | 1.9         | good          |
| 27                | Dimethyl acetamide | 20                                                 | 76                   | "             | 0.48                                   | 2.62                                      | 1<br>5.4  | 50                     | 2.5         | "             |
| 28                | Dimethyl acetamide | 25                                                 | 210                  | "             | 0.46                                   | 2.48                                      | 1<br>5.4  | 48                     | 2.7         | "             |
| 29                | Dimethyl acetamide | 30                                                 | 640                  | "             | 0.47                                   | 2.24                                      | 1<br>4.8  | 49                     | 2.6         | "             |
| 30                | Dimethyl acetamide | 35                                                 | >1,000               | somewhat poor | 0.43                                   | 1.96                                      | 1<br>4.6  | 45                     | 2.4         | somewhat poor |
| 31                | Dimethyl acetamide | 40                                                 | gelled               | poor          | 0.42                                   | 1.86                                      | 1<br>4.4  | 44                     | 2.1         | poor          |
| 32                | Dimethyl formamide | 10                                                 | 5.6                  | good          | 0.56                                   | 18.4                                      | 1<br>32.8 | 56                     | 2.1         | somewhat poor |
| 33                | Dimethyl formamide | 15                                                 | 15                   | "             | 0.49                                   | 2.70                                      | 1<br>5.5  | 52                     | 2.6         | good          |
| 34                | Dimethyl formamide | 20                                                 | 50                   | "             | 0.46                                   | 2.35                                      | 1<br>5.1  | 48                     | 2.6         | "             |
| 35                | Dimethyl formamide | 25                                                 | 140                  | "             | 0.47                                   | 2.31                                      | 1<br>4.9  | 49                     | 2.7         | "             |
| 36                | Dimethyl formamide | 30                                                 | 420                  | "             | 0.46                                   | 2.26                                      | 1<br>4.9  | 48                     | 2.9         | "             |
| 37                | Dimethyl formamide | 35                                                 | 1,200                | somewhat poor | 0.41                                   | 2.95                                      | 1<br>7.2  | 43                     | 2.7         | somewhat poor |
| 38                | Dimethyl formamide | 40                                                 | gelled               | poor          | 0.43                                   | 2.75                                      | 1<br>6.4  | 45                     | 2.6         | poor          |
| 39                | Dimethyl sulfoxide | 10                                                 | 15                   | good          | 0.50                                   | 16.1                                      | 1<br>32.2 | 49                     | 2.3         | somewhat poor |
| 40                | Dimethyl sulfoxide | 15                                                 | 44                   | "             | 0.46                                   | 3.15                                      | 1<br>6.8  | 47                     | 2.4         | good          |
| 41                | Dimethyl sulfoxide | 20                                                 | 130                  | "             | 0.44                                   | 2.15                                      | 1<br>4.9  | 46                     | 2.7         | "             |
| 42                | Dimethyl sulfoxide | 25                                                 | 390                  | "             | 0.45                                   | 2.35                                      | 1<br>5.2  | 48                     | 2.6         | "             |
| 43                | Dimethyl sulfoxide | 30                                                 | 1,100                | "             | 0.43                                   | 2.21                                      | 1<br>5.1  | 45                     | 2.4         | "             |
| 44                | Dimethyl sulfoxide | 35                                                 | gelled               | somewhat poor | 0.39                                   | 2.16                                      | 1<br>5.5  | 41                     | 2.3         | somewhat poor |

TABLE 3-continued

| Experiment number | Solvent            | Spinning Solution                                  |                      |           | Fiber Property                                 |                                           |          |                                 |                   |             |
|-------------------|--------------------|----------------------------------------------------|----------------------|-----------|------------------------------------------------|-------------------------------------------|----------|---------------------------------|-------------------|-------------|
|                   |                    | Concen-<br>tration of<br>polymer<br>mixture<br>(%) | Viscosity<br>(poise) | Stability | Void<br>Porosity,<br>V<br>(cm <sup>3</sup> /g) | Surface<br>area, A<br>(m <sup>2</sup> /g) | V/A      | Water<br>absorp-<br>tion<br>(%) | Strength<br>(g/d) | Operability |
| 45                | Dimethyl sulfoxide | 40                                                 | gelled               | poor      | 0.36                                           | 2.03                                      | 1<br>5.6 | 38                              | 2.0               | poor        |

## EXAMPLE 4

A polymer mixture consisting of 90 parts of an acrylic polymer, which had a composition of AN:MA:S-MAS=90.5:9.0:0.5(%), and 10 parts of cellulose acetate was dissolved in DMF to prepare a spinning solution containing 25% of the polymer mixture. The spinning solution was extruded from a spinneret into a coagulation bath consisting of 65% of DMF and 35% of water and kept at 25° C., and the extruded filaments were subjected to a primary drawing in various draw ratios shown in the following Table 4. The primarily drawn filaments were dried and after-treated under the same conditions as described in Example 1 to obtain 3-denier fibers. Properties of the resulting fibers are shown in Table 4.

15 A polymer mixture consisting of 90 parts of an acrylic polymer, which had a composition of AN:MA:S-MAS=92.5:7.0:0.5(%), and 10 parts of cellulose acetate was dissolved in DMF to prepare a spinning solution containing 25% of the polymer mixture, and the spinning solution was extruded from a spinneret into a coagulation bath consisting of 60% of DMF and 40% of water and kept at 30° C. The extruded filaments were subjected to a primary drawing to draw the filaments to 4.0 times their original length, and then dried until the water content of the filaments was decreased to not more than 0.5% by means of a hot roller type drier kept at a drying temperature shown in the following Table 5. The dried filaments were then subjected to a secondary

## EXAMPLE 5

TABLE 4

| Experiment number | Draw ratio in primary drawing | Void                                |                                        | Fiber property |                         |                                                              | Remarks            |
|-------------------|-------------------------------|-------------------------------------|----------------------------------------|----------------|-------------------------|--------------------------------------------------------------|--------------------|
|                   |                               | Porosity, V<br>(cm <sup>3</sup> /g) | Surface area, A<br>(m <sup>2</sup> /g) | V/A            | Water absorption<br>(%) | Others                                                       |                    |
| 46                | 1.5                           | 0.381                               | 3.05                                   | 1<br>8.0       | 40.3                    | dried filaments are brittle, and operability thereof is poor | Comparative sample |
| 47                | 2                             | 0.362                               | 2.01                                   | 1<br>5.6       | 38.5                    | dried filaments are brittle, and operability thereof is poor | Comparative sample |
| 48                | 3                             | 0.368                               | 1.99                                   | 1<br>5.4       | 39.0                    |                                                              | Present invention  |
| 49                | 4                             | 0.352                               | 2.01                                   | 1<br>5.7       | 37.5                    |                                                              | Present invention  |
| 50                | 5                             | 0.337                               | 1.71                                   | 1<br>5.1       | 36.1                    |                                                              | Present invention  |
| 51                | 6                             | 0.326                               | 1.58                                   | 1<br>4.8       | 35.0                    |                                                              | Present invention  |
| 52                | 7                             | 0.294                               | 1.75                                   | 1<br>6.0       | 32.0                    |                                                              | Present invention  |
| 53                | 8                             | 0.126                               | 0.84                                   | 1<br>6.7       | 16.0                    |                                                              | Present invention  |
| 54                | 9                             | 0.04                                | 0.28                                   | 1<br>7.0       | 8.0                     | yarn breakage occurs often                                   | Comparative sample |

60 drawing at 110° C. under wet heat to draw the filaments to 2 times their original length, and then mechanically crimped, and the crimps were set to obtain 3-denier fibers. Properties of the fibers are shown in Table 5.

TABLE 5

| Experiment number | Drying temperature (°C.) | Void                                |                                        |           | Fiber property          |                                         |                    |
|-------------------|--------------------------|-------------------------------------|----------------------------------------|-----------|-------------------------|-----------------------------------------|--------------------|
|                   |                          | Porosity, V<br>(cm <sup>3</sup> /g) | Surface area, A<br>(m <sup>2</sup> /g) | V/A       | Water absorption<br>(%) | Others                                  | Remarks            |
|                   | 55 60                    | 0.60                                | 26.4                                   | 1<br>44.0 | 56.1                    | poor in yarn property and in dyeability | Comparative sample |

TABLE 5-continued

| Experiment number | Drying temperature (°C.) | Void                             |                                     | Fiber property |                      |                                         | Remarks            |
|-------------------|--------------------------|----------------------------------|-------------------------------------|----------------|----------------------|-----------------------------------------|--------------------|
|                   |                          | Porosity, V (cm <sup>3</sup> /g) | Surface area, A (m <sup>2</sup> /g) | V/A            | Water absorption (%) | Others                                  |                    |
| 56                | 80                       | 0.57                             | 19.6                                | 1/34.1         | 50.3                 | poor in yarn property and in dyeability | Comparative sample |
| 57                | 100                      | 0.50                             | 7.5                                 | 1/15.0         | 51.6                 |                                         | Present invention  |
| 58                | 120                      | 0.41                             | 2.34                                | 1/5.7          | 43.0                 |                                         | Present invention  |
| 59                | 140                      | 0.35                             | 1.89                                | 1/5.4          | 37.3                 |                                         | Present invention  |
| 60                | 150                      | 0.30                             | 1.61                                | 1/5.4          | 32.6                 |                                         | Present invention  |
| 61                | 160                      | 0.25                             | 1.30                                | 1/5.2          | 27.8                 |                                         | Present invention  |
| 62                | 180                      | 0.23                             | 1.18                                | 1/5.1          | 25.9                 |                                         | Present invention  |
| 63                | 190                      | 0.21                             | 1.05                                | 1/5.0          | 24.0                 | fiber colors, and becomes rigid         | Comparative sample |
| 64                | 200                      | 0.21                             | 0.97                                | 1/4.6          | 24.0                 | fiber colors, and becomes rigid         | Comparative sample |

## EXAMPLE 6

A polymer mixture consisting of 85 parts of an acrylic polymer, which had a composition of AN:MA:SAS=89:10.4:0.6(%), and 15 parts of cellulose acetate was dissolved in DMF to prepare a spinning solution containing 27% of the polymer mixture, and the spinning solution was extruded from a spinneret into a coag-

30 kept at 125° C. to decrease the water content of the filaments to the water content shown in the following Table 6, and the dried filaments were subjected to the same aftertreatments as those described in Example 1 to obtain 2-denier fibers.

Properties of the fibers are shown in Table 6. Further, the fibers of Experiment Nos. 67 and 69 had ratios of microvoids of 15.3% and 14.2%, respectively.

TABLE 6

| Experiment number | Water content (%) | Void                             |                                     | Fiber property |                      |                                                       | Remarks            |
|-------------------|-------------------|----------------------------------|-------------------------------------|----------------|----------------------|-------------------------------------------------------|--------------------|
|                   |                   | Porosity, V (cm <sup>3</sup> /g) | Surface area, A (m <sup>2</sup> /g) | V/A            | Water absorption (%) | Others                                                |                    |
| 65                | 0                 | 0.433                            | 2.68                                | 1/6.2          | 45.2                 |                                                       | Present invention  |
| 66                | 0.1               | 0.457                            | 3.23                                | 1/7.1          | 47.5                 |                                                       | Present invention  |
| 67                | 0.2               | 0.505                            | 3.65                                | 1/8.0          | 52.1                 |                                                       | Present invention  |
| 68                | 0.3               | 0.546                            | 4.10                                | 1/7.5          | 56.0                 |                                                       | Present invention  |
| 69                | 0.5               | 0.582                            | 4.42                                | 1/7.6          | 59.4                 |                                                       | Present invention  |
| 70                | 1.0               | 0.648                            | 5.18                                | 1/8.0          | 65.7                 |                                                       | Present invention  |
| 71                | 2.0               | 0.694                            | 27.76                               | 1/40.0         | 70.1                 | low strength and poor dyeability, and uneven property | Comparative sample |
| 72                | 5.0               | 0.717                            | 29.5                                | 1/41.1         | 72.3                 | low strength and poor dyeability, and uneven property | Comparative sample |

ulation bath consisting of 70% of DMF and 30% of water and kept at 30° C. The extruded filaments were 65 subjected to a primary drawing to draw the filaments to 5 times their original length, and the primarily drawn filaments were dried by means of a hot roller type drier

## EXAMPLE 7

The same spinning solution as that used in Example 6 was extruded from a spinneret into a coagulation bath

consisting of 65% of DMF and 35% of water and kept at 25° C., and the extruded filaments were subjected to a primary drawing to draw the filaments to 4 times their original length. Then, the primarily drawn filaments were dried by means of a hot roller type drier kept at 125° C. until the water content of the filaments was

decreased to not more than 0.7%. The dried filaments were subjected to a secondary drawing under the same secondary drawing conditions as described in Example 5 and then mechanically crimped, and the crimps were set to obtain 3-denier fibers. Properties of the fibers are shown in the following Table 7.

TABLE 7(a)

| Experiment number | Secondary drawing condition |            | Porosity, V (cm <sup>3</sup> /g) | Surface area, A (m <sup>2</sup> /g) | V/A    | Fiber property       |                      | Remarks           |
|-------------------|-----------------------------|------------|----------------------------------|-------------------------------------|--------|----------------------|----------------------|-------------------|
|                   | Temperature (°C.)           | Draw ratio |                                  |                                     |        | Water absorption (%) | Others               |                   |
| 73                | 100                         | 0.9        | 0.333                            | 2.18                                | 1/6.6  | 35.7                 |                      | Present invention |
| 74                | "                           | 1.0        | 0.334                            | 2.20                                | 1/6.6  | 36.8                 |                      | Present invention |
| 75                | "                           | 1.5        | 0.338                            | 2.24                                | 1/6.6  | 36.2                 |                      | Present invention |
| 76                | "                           | 2          | 0.297                            | 2.32                                | 1/7.8  | 32.3                 |                      | Present invention |
| 77                | "                           | 3          | 0.222                            | 2.50                                | 1/11.2 | 25.1                 | yarn breakage occurs | Present invention |
| 78                | 110                         | 0.9        | 0.326                            | 2.08                                | 1/6.4  | 35.0                 |                      | Present invention |
| 79                | "                           | 1.0        | 0.359                            | 2.12                                | 1/6.0  | 37.0                 |                      | Present invention |
| 80                | "                           | 2          | 0.332                            | 2.16                                | 1/6.6  | 35.6                 |                      | Present invention |

TABLE 7(b)

| Experiment number | Secondary drawing condition |            | Porosity, V (cm <sup>3</sup> /g) | Surface area, A (m <sup>2</sup> /g) | V/A    | Fiber property       |                        | Remarks            |
|-------------------|-----------------------------|------------|----------------------------------|-------------------------------------|--------|----------------------|------------------------|--------------------|
|                   | Temperature (°C.)           | Draw ratio |                                  |                                     |        | Water absorption (%) | Others                 |                    |
| 81                | 110                         | 3          | 0.294                            | 2.24                                | 1/7.6  | 32.0                 | yarn breakage occurs   | Present invention  |
| 82                | "                           | 4          | 0.158                            | 2.44                                | 1/15.4 | 19.0                 | frequent yarn breakage | Comparative sample |
| 83                | 120                         | 0.8        | 0.286                            | 1.80                                | 1/6.2  | 31.2                 |                        | Present invention  |
| 84                | "                           | 1          | 0.323                            | 1.82                                | 1/5.6  | 34.8                 |                        | Present invention  |
| 85                | "                           | 2          | 0.329                            | 1.84                                | 1/5.6  | 35.1                 |                        | Present invention  |
| 86                | "                           | 3          | 0.297                            | 2.02                                | 1/6.8  | 32.3                 |                        | Present invention  |
| 87                | "                           | 4          | 0.169                            | 2.46                                | 1/14.6 | 20.1                 | yarn breakage occurs   | Comparative sample |
| 88                | "                           | 5          | —                                | —                                   | —      | —                    | spinning is impossible | Comparative sample |

TABLE 7(c)

| Experiment number | Secondary drawing condition |            | Porosity, V (cm <sup>3</sup> /g) | Surface area, A (m <sup>2</sup> /g) | V/A   | Fiber property       |        | Remarks           |
|-------------------|-----------------------------|------------|----------------------------------|-------------------------------------|-------|----------------------|--------|-------------------|
|                   | Temperature (°C.)           | Draw ratio |                                  |                                     |       | Water absorption (%) | Others |                   |
| 89                | 130                         | 0.8        | 0.295                            | 1.52                                | 1/5.2 | 32.0                 |        | Present invention |
| 90                | "                           | 1          | 0.339                            | 1.50                                | 1/4.4 | 36.0                 |        | Present invention |

TABLE 7(c)-continued

| Experiment number | Secondary drawing condition |            | Porosity, V (cm <sup>3</sup> /g) | Surface area, A (m <sup>2</sup> /g) | V/A    | Fiber property       |                        | Remarks            |
|-------------------|-----------------------------|------------|----------------------------------|-------------------------------------|--------|----------------------|------------------------|--------------------|
|                   | Temperature (°C.)           | Draw ratio |                                  |                                     |        | Water absorption (%) | Others                 |                    |
| 91                | "                           | 2          | 0.327                            | 1.60                                | 1/4.8  | 35.1                 |                        | Present invention  |
| 92                | "                           | 3          | 0.280                            | 1.80                                | 1/6.4  | 30.7                 |                        | Present invention  |
| 93                | "                           | 4          | 0.173                            | 2.04                                | 1/12.8 | 20.4                 | yarn breakage occurs   | Comparative sample |
| 94                | "                           | 5          | —                                | —                                   | —      | —                    | spinning is impossible | Comparative sample |

## EXAMPLE 8

A polymer mixture consisting of 80 parts of an acrylic polymer, which had a composition of AN:MA:SMAS=90.5:9.0:0.5(%), and 20 parts of cellulose acetate was dissolved in DMF to prepare a DMF solution containing 20% of the polymer mixture. Then, 100 parts of the DMF solution was mixed with 2 parts of water to prepare a spinning solution, and the spinning solution was extruded from a spinneret into a coagulation bath consisting of 50% of DMF and 50% of water and kept at 25° C. The extruded filaments were washed with water and then subjected to a primary drawing in hot water to draw the filaments to 4 times their original length. The primarily drawn filaments was dried until the water content of the filaments was decreased to not more than 1.0% by means of a hot roller type drier kept at 135° C. The dried filaments were subjected to a secondary drawing at 115° C. under wet heat to draw the filaments to 2 times their original length and then mechanically crimped, and the crimps were set to obtain 3-denier fibers.

The resulting fiber was a somewhat dull porous acrylic fiber having voids and having a porosity V of 0.3 cm<sup>3</sup>/g and a surface area A of voids of 1.03 m<sup>2</sup>/g, the ratio V/A being 1/3.43. The porous acrylic fiber had the following yarn properties; that is, a fineness of 2 deniers, a strength in dried state of 2.9 g/d and an elongation in dried state of 30.5%. Further, the fiber had a strength in wet state of 2.87 g/d and an elongation in wet state of 31.3%. Therefore, the yarn property of the fiber in the dried state was maintained in the wet state.

## EXAMPLE 9

A polymer mixture consisting of (100-X) parts of an acrylic polymer, which had a composition of AN:MA:SMAS=90.5:9.0:0.5(%), and X parts of cellulose acetate was dissolved in DMF to prepare a spinning solution containing 23% of the polymer mixture. The spinning solution was extruded from a spinneret into a coagulation bath consisting of 65% of DMF and 35% of water and kept at 20° C. The extruded filaments were subjected to a primary drawing to draw the filaments to 5 times their original length, and the primarily drawn

filaments were washed with water and dried until the water content of the filaments was decreased to 0.5% by means of a hot roller type drier kept at 120° C. The dried filaments were then subjected to a secondary drawing at 110° C. under wet heat to draw the filaments to 1.2 times their original length and then mechanically crimped, and the crimps were set to obtain 2-denier fibers.

For comparison, in Experiment No. 98, the above described polymer mixture was dissolved in DMF to prepare a spinning solution containing 23% of the polymer mixture, and the spinning solution was extruded from a spinneret into a coagulation bath consisting of 65% of DMF and 35% of water and kept at 40° C. The extruded filaments were subjected to a primary drawing to draw the filaments to 6 times their original length, and the primarily drawn filaments were washed with water, subjected to a heat treatment at 125° C. under wet heat without drawing and shrinking, and then dried. The dried filaments were mechanically crimped, and the crimps were set to obtain 2-denier fibers. In experiment No. 99, the above described acrylic polymer alone was dissolved in DMF to prepare a spinning solution containing 23% of the acrylic polymer alone, and the spinning solution was extruded from a spinneret into a coagulation bath consisting of 65% of DMF and 35% of water and kept at 40° C. The extruded filaments were subjected to a primary drawing to draw the filaments to 5 times their original length, and the primarily drawn filaments were washed with water, subjected to a secondary drawing at 110° C. under wet heat to draw the filaments to 1.2 times their original length, and then dried in the same manner as described above. The dried filaments were mechanically crimped and the crimps were set to obtain 2-denier fibers.

Properties of the fibers are shown in the following Table 8. The dyeability (depth and brilliancy) was evaluated by the depth of color when a black dye was deposited on the fiber in an amount of 4.5% based on the amount of the fiber. In the evaluation of the dyeability, the depth of color of commercially available acrylic fiber (Kanebo Acryl Regular type) is graded as 5th grade. The larger the value, the more the sample fiber has a deeper and more brilliant color.

TABLE 8

| Experiment number | Polymer mixture X (parts) | Ratio of microvoid (%) | Yarn property        |                |                | Dyeability (depth and brilliancy) (grade) | Remarks           |
|-------------------|---------------------------|------------------------|----------------------|----------------|----------------|-------------------------------------------|-------------------|
|                   |                           |                        | Water absorption (%) | Strength (g/d) | Elongation (%) |                                           |                   |
| 95                | 4                         | 10.2                   | 21                   | 3.6            | 39             | 4                                         | Present invention |

TABLE 8-continued

| Experiment number | Polymer mixture<br>(parts) | X<br>(parts) | Ratio of<br>microvoid<br>(%) | Water<br>absorption<br>(%) | Yarn property     |                   | Dyeability<br>(depth and<br>brilliancy)<br>(grade) | Remarks |
|-------------------|----------------------------|--------------|------------------------------|----------------------------|-------------------|-------------------|----------------------------------------------------|---------|
|                   |                            |              |                              |                            | Strength<br>(g/d) | Elongation<br>(%) |                                                    |         |
| 96                | 10                         | 12.4         | 38                           | 3.2                        | 36                | 4                 | Present invention                                  |         |
| 97                | 15                         | 16.0         | 43                           | 3.0                        | 33                | 3~4               | Present invention                                  |         |
| 98                | 4                          | 78.6         | 24                           | 2.2                        | 26                | 1~2               | Comparative sample                                 |         |
| 99                | 0                          | 44.9         | 9                            | 2.5                        | 32                | 2                 | Comparative sample                                 |         |

## EXAMPLE 10

A polymer mixture consisting of 85 parts of an acrylic polymer (I), which had a composition of AN:MA:S-MAS=90.5:9.0:0.5(%), 15 parts of cellulose acetate (II), and a variable amount of an acrylic copolymer (III), which had a composition of AN:CH<sub>2</sub>=CH—COO—(CH<sub>2</sub>CH<sub>2</sub>O)<sub>n</sub>CH<sub>3</sub>=85:15(%), was dissolved in DMF to prepare a spinning solution containing 23% of the polymer mixture. The spinning solution was extruded from a spinneret into a coagulation bath consisting of 56% of DMF and 44% of water and kept at 20° C., and the extruded filaments were subjected to a primary drawing to draw the filaments to 5 times their original length. The primarily drawn filaments were dried until the water content in the filaments was decreased to 0.7% by means of a hot roller type drier kept at 120° C., and then subjected to a secondary drawing at 100° C. under wet heat to draw the filaments to 1.1 times their original length. The filaments were mechanically crimped, and the crimps were set to obtain 3-denier fibers. Properties of the fibers are shown in the following Table 9.

## EXAMPLE 11

A polymer mixture consisting of 85 parts of an acrylic polymer (I), which had a composition of AN:MA:S-SAS=90.3:9.0:0.7(%), 15 parts of cellulose acetate (II) and 2 parts of an acrylic copolymer (III), which was a copolymer of 90% of AN and 10% of a monomer shown by the following general formula, was dissolved in DMF to prepare a spinning solution containing 27% of the polymer mixture. The extrusion of the spinning solution, and the after-treatment of the extruded filaments were carried out under the same condition as described in Example 10 to obtain 3-denier fibers.

The general formula of the above described monomer is as follows:



wherein X represents R<sub>2</sub> or



(R<sub>2</sub>, R<sub>3</sub>, 1 and m are shown in the following Table 10).

Properties of the resulting fibers are shown in Table 10.

TABLE 9

| Experiment number | Polymer mixture<br>(parts) |      |       | Void                                   |                                           | Fiber property   |                            |                                     |                    |
|-------------------|----------------------------|------|-------|----------------------------------------|-------------------------------------------|------------------|----------------------------|-------------------------------------|--------------------|
|                   | [I]                        | [II] | [III] | Porosity,<br>V<br>(cm <sup>3</sup> /g) | Surface<br>area, A<br>(m <sup>2</sup> /g) | V/A              | Water<br>absorption<br>(%) | Others                              | Remarks            |
| 100               | 85                         | 15   | 0.5   | 0.41                                   | 2.01                                      | <u>1</u><br>4.9  | 43                         | good in luster<br>and in dyeability | Present invention  |
| 101               | "                          | "    | 2     | 0.40                                   | 1.97                                      | <u>1</u><br>4.9  | 43                         | good in luster<br>and in dyeability | Present invention  |
| 102               | "                          | "    | 5     | 0.39                                   | 1.95                                      | <u>1</u><br>5.0  | 40                         | good in luster<br>and in dyeability | Present invention  |
| 103               | "                          | "    | 10    | 0.34                                   | 1.96                                      | <u>1</u><br>5.8  | 36                         | good in luster<br>and in dyeability | Present invention  |
| 104               | "                          | "    | 30    | 0.26                                   | 1.74                                      | <u>1</u><br>6.7  | 29                         | good in luster<br>and in dyeability | Present invention  |
| 105               | "                          | "    | 50    | 0.16                                   | 1.03                                      | <u>1</u><br>6.4  | 17                         | good in luster<br>and in dyeability | Present invention  |
| 106               | "                          | "    | 60    | 0.03                                   | 0.36                                      | <u>1</u><br>12.0 | 5                          | poor heat resistance                | Comparative sample |

TABLE 10

| Experiment number | Monomer        |                 |    |    | Porosity, V (cm <sup>3</sup> /g) | Surface area, A (m <sup>2</sup> /g) | Fiber property |                      |                                                 |
|-------------------|----------------|-----------------|----|----|----------------------------------|-------------------------------------|----------------|----------------------|-------------------------------------------------|
|                   | R <sub>2</sub> | R <sub>3</sub>  | 1  | m  |                                  |                                     | V/A            | Water absorption (%) | Others                                          |
| 107               | H              | —               | —  | —  | 0.34                             | 1.51                                | 1<br>4.4       | 35                   | good in luster and dyeability Present invention |
| 108               | —              | H               | 8  | 0  | 0.40                             | 1.99                                | 1<br>5.0       | 43                   | good in luster and dyeability Present invention |
| 109               | —              | H               | 0  | 15 | 0.42                             | 2.10                                | 1<br>5.0       | 44                   | good in luster and dyeability Present invention |
| 110               | —              | CH <sub>3</sub> | 10 | 15 | 0.43                             | 2.15                                | 1<br>5.0       | 46                   | good in luster and dyeability Present invention |
| 111               | —              | H               | 20 | 20 | 0.45                             | 2.17                                | 1<br>4.8       | 48                   | good in luster and dyeability Present invention |

## EXAMPLE 12

A polymer mixture consisting of 90 parts of an acrylic polymer, which had a composition of AN:MA:SMAS=90.5:9.0:0.5(%), and 10 parts of cellulose acetate was dissolved in DMF to prepare a spinning solution containing 23% of the polymer mixture. The spinning solution was extruded from a spinneret into a coagulation bath consisting of 60% of DMF and 40% of water and kept at a temperature shown in the following Table 11, and then the extruded filaments were subjected to a primary drawing to draw the filaments to 5 times their original length. The primarily drawn filaments were washed with water, dried so that the water content of the filaments would be decreased to not more than 1%, and then subjected to a secondary drawing at 110° C. under wet heat to draw the filaments to 1.4 times their original length. The secondarily drawn filaments were mechanically crimped, and the crimps were set to obtain 2-denier fibers. Properties of the fibers are shown in the following Table 11.

The fiber of Experiment No. 114 had a porosity of 1.10 cm<sup>3</sup>/g before drying, a porosity of 0.213 cm<sup>3</sup>/g after drying (before secondary drawing), and a porosity of 0.336 cm<sup>3</sup>/g after secondary drawing.

20

## EXAMPLE 13

A polymer component A consisting of (100-C) parts of an acrylic polymer, which had a composition of AN:MA:SMAS=90.6:9.0:0.4(%), and C parts of cellulose acetate was dissolved in DMF to prepare a spinning solution A containing 22% of the polymer component A. A polymer component B consisting of the same acrylic polymer as used in the polymer component A was dissolved in DMF to prepare a spinning solution B containing 22% of the polymer component B. The spinning solutions A and B were extruded in a conjugate ratio of 5/5 (weight ratio) from a spinneret designed for side-by-side conjugate spinning into a coagulation bath consisting of a 65% DMF aqueous solution kept at 20° C.

The extruded filaments were subjected to a primary drawing to draw the filaments to 6 times their original length. The primarily drawn filaments were dried by means of a hot roller type drier kept at 120° C. until the water content of the filaments was decreased to 0.7%, and then subjected to a secondary drawing at 100° C. under wet heat to draw the filaments to 1.1 times their original length. The secondarily drawn filaments were mechanically crimped, and the crimps were set to obtain 3-denier fibers. The resulting acrylic composite fibers had substantially no latent crimpability. Properties of the fibers are shown in the following Table 12.

TABLE 11

| Experiment number | Coagulation bath temperature (°C.) | Ratio of microvoid (%) | Fiber property       |                |                |                        |               |                    | Remarks |  |
|-------------------|------------------------------------|------------------------|----------------------|----------------|----------------|------------------------|---------------|--------------------|---------|--|
|                   |                                    |                        | Water absorption (%) | Yarn property  |                | Dyeability             |               |                    |         |  |
|                   |                                    |                        |                      | Strength (g/d) | Elongation (%) | (depth and brilliancy) | (grade)       | Heat resistance    |         |  |
| 112               | 10                                 | 7.8                    | 38                   | 3.4            | 37             | 4                      | good          | Present invention  |         |  |
| 113               | 15                                 | 7.7                    | 35                   | 3.3            | 39             | 4                      | "             | Present invention  |         |  |
| 114               | 20                                 | 11.8                   | 37                   | 3.2            | 38             | 4                      | "             | Present invention  |         |  |
| 115               | 25                                 | 15.7                   | 39                   | 3.2            | 37             | 3~4                    | "             | Present invention  |         |  |
| 116               | 30                                 | 19.3                   | 41                   | 3.1            | 34             | 3                      | "             | Present invention  |         |  |
| 117               | 35                                 | 34.0                   | 43                   | 2.7            | 29             | 2                      | somewhat poor | Comparative sample |         |  |
| 118               | 40                                 | 49.0                   | 45                   | 2.4            | 25             | 1~2                    | poor          | Comparative sample |         |  |

TABLE 12

| Experiment number | Polymer component A C (parts) | Fiber property                |                                  |                      |               |             |                                             | Remarks            |
|-------------------|-------------------------------|-------------------------------|----------------------------------|----------------------|---------------|-------------|---------------------------------------------|--------------------|
|                   |                               | Void                          |                                  | Water absorption (%) |               | Dyeability  | Others                                      |                    |
|                   |                               | Porosity (cm <sup>3</sup> /g) | Surface area (m <sup>2</sup> /g) |                      |               |             |                                             |                    |
| 119               | 0                             | 0.00                          | 0.00                             | 4                    | good          | good luster |                                             | Comparative sample |
| 120               | 1                             | 0.021                         | 0.28                             | 6                    | "             | "           |                                             | Comparative sample |
| 121               | 2                             | 0.074                         | 0.72                             | 11                   | "             | "           |                                             | Present invention  |
| 122               | 5                             | 0.137                         | 0.88                             | 17                   | "             | "           |                                             | Present invention  |
| 123               | 10                            | 0.221                         | 1.02                             | 25                   | "             | "           |                                             | Present invention  |
| 124               | 20                            | 0.305                         | 1.22                             | 33                   | "             | "           |                                             | Present invention  |
| 125               | 40                            | 0.609                         | 1.58                             | 62                   | "             | "           |                                             | Present invention  |
| 126               | 50                            | 0.714                         | 1.83                             | 72                   | somewhat poor | "           |                                             | Present invention  |
| 127               | 60                            | 0.924                         | 2.16                             | 92                   | poor          | poor        | poor yarn property and somewhat poor luster | Comparative sample |

## EXAMPLE 14

A polymer component A consisting of (100-C) parts of an acrylic polymer, which had a composition of AN:AM:SMAS=90.6:9.0:0.4(%), and C parts of cellulose acetate was dissolved in DMF to prepare a spinning solution A containing 22% of the polymer component A. A polymer component B consisting of an acrylic polymer having a composition of AN:MA:SMAS=90.4:9.0:0.6(%) was dissolved in DMF to prepare a spinning solution B containing 22% of the poly-

mer component B. The spinning solutions A and B were extruded in various conjugate ratios from a spinneret, which was designed for bonding the spinning solutions A and B in a side-by-side relation, into a coagulation bath consisting of a 65% DMF aqueous solution kept at 20° C. Then, the extruded filaments were subjected to after-treatments in the same manner as described in Example 13 to obtain 3-denier acrylic composite fibers. Properties of the composite fibers are shown in the following Table 13. The resulting composite fibers had substantially no latent crimpability.

TABLE 13(a)

| Experiment number | Polymer component A C (parts) | Conjugate ratio of A/B (weight ratio) | Fiber property                |                                  |                |               | Remarks                        |
|-------------------|-------------------------------|---------------------------------------|-------------------------------|----------------------------------|----------------|---------------|--------------------------------|
|                   |                               |                                       | Void                          |                                  | Water          |               |                                |
|                   |                               |                                       | Porosity (cm <sup>3</sup> /g) | Surface area (m <sup>2</sup> /g) | Absorption (%) | Dyeability    | Others                         |
| 128               | 2                             | 1/9                                   | 0.01                          | 0.17                             | 4              | good          | poor water absorption          |
| 129               | 2                             | 2/8                                   | 0.03                          | 0.33                             | 6              | "             | somewhat poor water            |
| 130               | 2                             | 3/7                                   | 0.04                          | 0.49                             | 7              | "             | somewhat poor water absorption |
| 131               | 2                             | 5/5                                   | 0.06                          | 0.81                             | 12             | "             | somewhat poor water absorption |
| 132               | 2                             | 7/3                                   | 0.09                          | 0.93                             | 12             | "             | somewhat poor water absorption |
| 133               | 2                             | 8/2                                   | 0.10                          | 1.07                             | 13             | "             | somewhat poor water absorption |
| 134               | 2                             | 9/1                                   | 0.12                          | 1.46                             | 14             | somewhat poor | somewhat poor water absorption |
| 135               | 10                            | 1/9                                   | 0.03                          | 0.21                             | 4              | good          | poor water absorption          |
| 136               | 10                            | 2/8                                   | 0.07                          | 0.41                             | 13             | "             |                                |
| 137               | 10                            | 3/7                                   | 0.13                          | 0.63                             | 17             | "             |                                |
| 138               | 10                            | 5/5                                   | 0.24                          | 1.02                             | 27             | "             |                                |

TABLE 13(b)

| Experiment number | Polymer component A C (parts) | Conjugate ratio of A/B (weight ratio) | Fiber property                |                                  |                |            | Remarks |
|-------------------|-------------------------------|---------------------------------------|-------------------------------|----------------------------------|----------------|------------|---------|
|                   |                               |                                       | Void                          |                                  | Water          |            |         |
|                   |                               |                                       | Porosity (cm <sup>3</sup> /g) | Surface area (m <sup>2</sup> /g) | Absorption (%) | Dyeability | Others  |
| 139               | 10                            | 6/4                                   | 0.25                          | 1.22                             | 28             | good       | Present |

TABLE 13(b)-continued

| Experiment number | Polymer component A C (parts) | Conjugate ratio of A/B (weight ratio) | Fiber property                |                                  |                |               |                       | Remarks            |  |
|-------------------|-------------------------------|---------------------------------------|-------------------------------|----------------------------------|----------------|---------------|-----------------------|--------------------|--|
|                   |                               |                                       | Void                          |                                  | Water          |               |                       |                    |  |
|                   |                               |                                       | Porosity (cm <sup>3</sup> /g) | Surface area (m <sup>2</sup> /g) | Absorption (%) | Dyeability    | Others                |                    |  |
| 140               | 10                            | 7/3                                   | 0.29                          | 1.44                             | 32             | "             | "                     | invention          |  |
| 141               | 10                            | 8/2                                   | 0.32                          | 1.63                             | 35             | somewhat poor | somewhat poor luster  | Present invention  |  |
| 142               | 10                            | 9/1                                   | 0.38                          | 1.84                             | 41             | poor          | poor luster           | Comparative sample |  |
| 143               | 30                            | 1/9                                   | 0.06                          | 0.28                             | 7              | good          | poor water absorption | Comparative sample |  |
| 144               | "                             | 2/8                                   | 0.12                          | 0.54                             | 14             | "             | "                     | Present invention  |  |
| 145               | "                             | 3/7                                   | 0.18                          | 0.83                             | 21             | "             | "                     | Present invention  |  |
| 146               | "                             | 5/5                                   | 0.24                          | 1.39                             | 33             | "             | "                     | Present invention  |  |
| 147               | "                             | 6/4                                   | 0.35                          | 1.68                             | 39             | "             | "                     | Present invention  |  |
| 148               | "                             | 7/3                                   | 0.41                          | 1.91                             | 42             | somewhat poor | somewhat poor luster  | Present invention  |  |
| 149               | "                             | 8/2                                   | 0.47                          | 2.20                             | 49             | somewhat poor | "                     | Present invention  |  |

TABLE 13(c)

| Experiment number | Polymer component A C (parts) | Conjugate ratio of A/B (weight ratio) | Fiber property                |                                  |                |               |                                     | Remarks            |  |
|-------------------|-------------------------------|---------------------------------------|-------------------------------|----------------------------------|----------------|---------------|-------------------------------------|--------------------|--|
|                   |                               |                                       | Void                          |                                  | Water          |               |                                     |                    |  |
|                   |                               |                                       | Porosity (cm <sup>3</sup> /g) | Surface area (m <sup>2</sup> /g) | Absorption (%) | Dyeability    | Others                              |                    |  |
| 150               | 30                            | 9/1                                   | 0.53                          | 2.48                             | 54             | poor          | poor luster                         | Comparative sample |  |
| 151               | 50                            | 1/9                                   | 0.04                          | 0.31                             | 10             | good          | poor water absorption               | Comparative sample |  |
| 152               | "                             | 2/8                                   | 0.24                          | 0.74                             | 27             | "             | "                                   | Present invention  |  |
| 153               | "                             | 3/7                                   | 0.39                          | 1.12                             | 43             | "             | "                                   | Present invention  |  |
| 154               | "                             | 5/5                                   | 0.68                          | 1.86                             | 71             | "             | "                                   | Present invention  |  |
| 155               | "                             | 6/4                                   | 0.79                          | 2.23                             | 85             | somewhat poor | somewhat poor luster                | Comparative sample |  |
| 156               | "                             | 7/3                                   | 0.97                          | 2.61                             | 97             | somewhat poor | poor in luster and in yarn property | Comparative sample |  |
| 157               | "                             | 8/2                                   | 1.07                          | 2.98                             | 110            | poor          | poor in luster and in yarn property | Comparative sample |  |
| 158               | "                             | 9/1                                   | 1.21                          | 3.38                             | 126            | "             | poor in luster and in yard property | Comparative sample |  |

## EXAMPLE 15

A polymer component A consisting of 85 parts of an acrylic polymer, which had a composition of AN:MA:SMAS=90.4:9.0:0.6(%), and 15 parts of cellulose acetate was dissolved in DMF to prepare a spinning solution A containing 22% of the polymer component A. A polymer component B consisting of the same acrylic polymer as used in the polymer component A was dissolved in DMF to prepare a spinning solution B containing 22% of the polymer component B. The spinning solutions A and B were extruded from a spinneret in a side-by-side relation and in a conjugate ratio (weight ratio) of component A/component B of 5/5 into a coagulation bath consisting of 60% of DMF and

40% of water and kept at a temperature shown in the following Table 14. The extruded filaments were subjected to a primary drawing to draw the filaments to 5 times their original length. Then, the primarily drawn filaments were washed with water, dried by means of a hot roller type drier kept at 120° C. until the water content of the filaments was decreased to not more than 1%, and then subjected to a secondary drawing at 110° C. under wet heat to draw the filaments to 1.2 times their original length. The secondarily drawn filaments were mechanically crimped and the crimps were set to obtain 2-denier composite fibers. Properties of the fibers are shown in Table 14. The evaluation of the dyeability was carried out in the same manner as described in Example 9.

TABLE 14

| Experiment number | Coagulation bath temperature (°C.) | Ratio of microvoid (%) | Water absorption (%) | Fiber property |                | Dyeability (depth and brilliancy) (grade) | Remarks            |
|-------------------|------------------------------------|------------------------|----------------------|----------------|----------------|-------------------------------------------|--------------------|
|                   |                                    |                        |                      | Strength (g/d) | Elongation (%) |                                           |                    |
| 159               | 10                                 | 7.4                    | 27                   | 3.5            | 41             | 4~5                                       | Present invention  |
| 160               | 15                                 | 7.2                    | 27                   | 3.3            | 39             | 4                                         | Present invention  |
| 161               | 20                                 | 11.3                   | 29                   | 3.4            | 38             | 4                                         | Present invention  |
| 162               | 25                                 | 15.1                   | 30                   | 3.2            | 34             | 4                                         | Present invention  |
| 163               | 30                                 | 19.7                   | 31                   | 3.0            | 33             | 3~4                                       | Present invention  |
| 164               | 35                                 | 35.6                   | 33                   | 2.6            | 28             | 2                                         | Comparative sample |
| 165               | 40                                 | 51.2                   | 32                   | 2.4            | 28             | 2                                         | Comparative sample |

## EXAMPLE 16

ity. Properties of the resulting composite fibers are shown in Table 15.

TABLE 15

| Experiment number | Draw ratio in primary drawing | Water absorption (%) | Fiber property     |                    |                                                       |  | Remarks            |
|-------------------|-------------------------------|----------------------|--------------------|--------------------|-------------------------------------------------------|--|--------------------|
|                   |                               |                      | Dyeability         | Others             | Operability                                           |  |                    |
| 166               | 2                             | 39.7                 | poor               | whitening          | yarn breakage occurs often after drying               |  | Comparative sample |
| 167               | 2.5                           | 39.4                 | substantially good | somewhat whitening |                                                       |  | Present invention  |
| 168               | 3                             | 37.5                 | good               | good yarn property | good crimp developing property                        |  | Present invention  |
| 169               | 4                             | 35.6                 | "                  | good yarn property | good crimp developing property                        |  | Present invention  |
| 170               | 6                             | 36.7                 | "                  | good yarn property | good crimp developing property                        |  | Present invention  |
| 171               | 8                             | 35.3                 | "                  | good yarn property | good crimp developing property                        |  | Present invention  |
| 172               | 9                             | 24.7                 | "                  | good yarn property | yarn breakage occurs often during the primary drawing |  | Comparative sample |
| 173               | 10                            | 16.5                 | somewhat poor      | uneven luster      | yarn breakage occurs often during the primary drawing |  | Comparative sample |

A polymer component A consisting of 80 parts of an acrylic polymer, which had a composition of AN:MA:SMAS=91.5:8.0:0.5(%), and 20 parts of cellulose acetate and a polymer component B consisting of an acrylic polymer, which had a composition of AN:MA:SMAS=89.0:10.5:0.5(%), were separately dissolved in DMF to prepare spinning solutions A and B containing 23% of the polymer components A and B, respectively. The spinning solutions A and B were extruded from a spinneret in a conjugate ratio (weight ratio) of component A/component B of 5/5 and in a side-by-side relation into a coagulation bath consisting of a 56% DMF aqueous solution kept at 20° C. The extruded filaments were subjected to a primary drawing in a draw ratio shown in the following Table 15. The primarily drawn filaments were washed with water, dried by means of a hot roller type drier kept at 125° C. until the water content of the filaments was decreased to 0.7%, and then subjected to a secondary drawing at 115° C. under wet heat to draw the filaments to 1.4 times their original length. The secondarily drawn filaments were mechanically crimped, and the crimps were set to obtain a composite fiber having latent crimpabil-

## EXAMPLE 17

A polymer component A consisting of 70 parts of an acrylic polymer, which had a composition of AN:MA:SMAS=90.6:9.0:0.4(%), and 30 parts of cellulose acetate, and a polymer component B consisting of the same acrylic polymer as used in the polymer component A, which had a composition of AN:MA:SMAS=90.6:9.0:0.4(%), was dissolved in DMF to prepare spinning solutions A and B containing 25% of the polymer components A and B, respectively. The spinning solutions A and B were extruded from a spinneret in a conjugate ratio (weight ratio) of component A/component B of 5/5 and in a side-by-side relation into a coagulation bath consisting of a 60% DMF aqueous solution kept at 25° C. The extruded filaments were subjected to a primary drawing to draw the filaments to 4 times their original length. The primarily drawn filaments were washed with water, dried by means of a hot roller type drier kept at a temperature shown in the following Table 16 until the water content of the filaments was decreased to not more than 0.8%, and then subjected to a secondary drawing at 105° C. under wet heat to draw the filaments to 1.6 times their original

length. The secondarily drawn filaments were mechanically crimped, and the crimps were set to obtain 3-denier composite fibers. Properties of the fibers are shown in Table 16.

TABLE 16

| Experiment number | Drying temperature (°C.) | Fiber property                |                                  |            |               |                                             | Remarks            |
|-------------------|--------------------------|-------------------------------|----------------------------------|------------|---------------|---------------------------------------------|--------------------|
|                   |                          | Void                          | Water absorption (%)             | Dyeability | Others        |                                             |                    |
|                   |                          | Porosity (cm <sup>3</sup> /g) | Surface area (m <sup>2</sup> /g) |            |               |                                             |                    |
| 174               | 60                       | 0.56                          | 19.4                             | 58         | poor          | yarn property is poor and fiber is whitened | Comparative sample |
| 175               | 80                       | 0.51                          | 16.3                             | 53         | "             | yarn property is poor and fiber is whitened | Comparative sample |
| 176               | 100                      | 0.46                          | 6.88                             | 49         | somewhat poor | yarn property is poor and fiber is whitened | Present invention  |
| 177               | 120                      | 0.42                          | 1.57                             | 46         | good          | yarn property is poor and fiber is whitened | Present invention  |
| 178               | 140                      | 0.37                          | 1.43                             | 40         | "             | yarn property is poor and fiber is whitened | Present invention  |
| 179               | 160                      | 0.31                          | 1.36                             | 34         | "             | yarn property is poor and fiber is whitened | Present invention  |
| 180               | 180                      | 0.26                          | 1.14                             | 27         | "             | fiber somewhat colors                       | Present invention  |
| 181               | 190                      | 0.21                          | 1.05                             | 24         | "             | fiber colors and becomes rigid              | Comparative sample |
| 182               | 200                      | 0.18                          | 0.91                             | 22         | somewhat poor | fiber colors and becomes rigid              | Comparative sample |

## EXAMPLE 18

The same water washed filament tows as those obtained in Example 17, which had been swollen with water, were dried by means of a hot roller type drier kept at 120° C. until the water content of the tows was decreased to various water contents shown in the following Table 17, and the dried tows were treated under the same after-treatment condition as described in Example 17 to obtain 3-denier fibers. Properties of the fibers are shown in Table 17.

30 The spinning solutions A and B were extruded from a spinneret in a conjugate ratio (weight ratio) of component A/component B of 5/5 and in a side-by-side relation into a coagulation bath consisting of a 60% DMF aqueous solution kept at 18° C. The extruded filaments were subjected to a primary drawing to draw the filaments to 5 times their original length. The primarily drawn filaments were washed with water, dried by means of a hot roller type drier kept at 120° C. while blowing hot air kept at 130° C. until the water content of the filaments was decreased to 0.7%, and then sub-  
35

TABLE 17

| Experiment number | Water content (%) | Fiber property                |                                  |            |               |                                        | Remarks            |
|-------------------|-------------------|-------------------------------|----------------------------------|------------|---------------|----------------------------------------|--------------------|
|                   |                   | Void                          | Water absorption (%)             | Dyeability | Others        |                                        |                    |
|                   |                   | Porosity (cm <sup>3</sup> /g) | Surface area (m <sup>2</sup> /g) |            |               |                                        |                    |
| 183               | 0.1               | 0.37                          | 1.28                             | 40         | good          |                                        | Present invention  |
| 184               | 0.3               | 0.39                          | 1.41                             | 42         | "             |                                        | Present invention  |
| 185               | 0.5               | 0.38                          | 1.34                             | 41         | "             |                                        | Present invention  |
| 186               | 0.7               | 0.41                          | 1.49                             | 43         | "             |                                        | Present invention  |
| 187               | 1.0               | 0.43                          | 2.48                             | 45         | "             |                                        | Present invention  |
| 188               | 1.1               | 0.53                          | 5.69                             | 54         | somewhat poor | uneven luster and uneven yarn property | Comparative sample |
| 189               | 1.5               | 0.76                          | 13.7                             | 78         | poor          | uneven luster and uneven yarn property | Comparative sample |
| 190               | 2.0               | 0.89                          | 16.4                             | 89         | "             | uneven luster and uneven yarn property | Comparative sample |
| 191               | 5.0               | 1.30                          | 23.1                             | 126        | "             | uneven luster and uneven yarn property | Comparative sample |

## EXAMPLE 19

A polymer component A consisting of 70 parts of an acrylic polymer, which had a composition of AN:MA:SMAS=90.5:9.0:0.5(%), and 30 parts of cellulose acetate, and a polymer component B consisting of an

65 jected to a secondary drawing under a condition shown in the following Table 18. The secondarily drawn filaments were mechanically crimped, and the crimps were set to obtain composite fibers having a latent crimpability. Properties of the fibers are shown in Table 18.

TABLE 18(a)

| Experiment number | Secondary drawing condition |            | Fiber property       |               |                                              |                    |  | Remarks           |
|-------------------|-----------------------------|------------|----------------------|---------------|----------------------------------------------|--------------------|--|-------------------|
|                   | Temperature (°C.)           | Draw ratio | Water absorption (%) | Dyeability    | Others                                       | Operability        |  |                   |
| 192               | 100                         | 0.9        | 39                   | good          | good luster                                  | good               |  | Present invention |
| 193               | "                           | 1.0        | 43                   | "             | "                                            | "                  |  | Present invention |
| 194               | "                           | 1.5        | 41                   | "             | "                                            | "                  |  | Present invention |
| 195               | "                           | 2          | 36                   | "             | "                                            | "                  |  | Present invention |
| 196               | "                           | 3          | 31                   | somewhat poor | somewhat poor in luster and in yarn property | some yarn breakage |  | Present invention |
| 197               | 110                         | 0.9        | 44                   | good          | good luster                                  | good               |  | Present invention |
| 198               | "                           | 1.0        | 45                   | "             | "                                            | "                  |  | Present invention |
| 199               | "                           | 1.5        | 41                   | "             | "                                            | "                  |  | Present invention |

TABLE 18(b)

| Experiment number | Secondary drawing condition |            | Fiber property       |               |                                              |                                             |  | Remarks            |
|-------------------|-----------------------------|------------|----------------------|---------------|----------------------------------------------|---------------------------------------------|--|--------------------|
|                   | Temperature (°C.)           | Draw ratio | Water absorption (%) | Dyeability    | Others                                       | Operability                                 |  |                    |
| 200               | 110                         | 2          | 38                   | good          | good luster                                  | good                                        |  | Present invention  |
| 201               | "                           | 3          | 31                   | somewhat poor | somewhat poor in luster and in yarn property | some yarn breakage                          |  | Present invention  |
| 202               | "                           | 4          | —                    | —             | —                                            | frequent yarn breakage and poor operability |  | Comparative sample |
| 203               | 120                         | 0.85       | 35                   | good          | good luster                                  | good                                        |  | Present invention  |
| 204               | "                           | 1.0        | 41                   | "             | "                                            | "                                           |  | Present invention  |
| 205               | "                           | 2          | 36                   | "             | "                                            | "                                           |  | Present invention  |

TABLE 18(c)

| Experiment number | Secondary drawing condition |            | Fiber property       |               |                                              |                        |  | Remarks            |
|-------------------|-----------------------------|------------|----------------------|---------------|----------------------------------------------|------------------------|--|--------------------|
|                   | Temperature (°C.)           | Draw ratio | Water absorption (%) | Dyeability    | Others                                       | Operability            |  |                    |
| 206               | 120                         | 3          | 29                   | somewhat poor | somewhat poor in luster and in yarn property | some yarn breakage     |  | Present invention  |
| 207               | "                           | 4          | 18                   | somewhat poor | somewhat poor in luster and in yarn property | frequent yarn breakage |  | Comparative sample |
| 208               | 130                         | 0.8        | 33                   | good          | good luster                                  | good                   |  | Present invention  |
| 209               | "                           | 1.0        | 35                   | "             | "                                            | "                      |  | Present invention  |
| 210               | "                           | 2          | 31                   | "             | "                                            | "                      |  | Present invention  |
| 211               | "                           | 3          | 25                   | somewhat poor | somewhat poor in luster and in yarn property | some yarn breakage     |  | Present invention  |
| 212               | "                           | 4          | 16                   | somewhat poor | somewhat poor in luster and in yarn property | frequent yarn breakage |  | Comparative sample |

## EXAMPLE 20

A polymer component A consisting of (100-C) parts of an acrylic polymer, which had a composition of AN:MA:SMAS=(99.5-y):y:0.5(%), and C parts of cel-

lulose acetate, and a polymer component B consisting of an acrylic polymer, which had a composition of AN:MA:SMAS=(99.5-y):y:0.5(%), were separately dissolved in DMF to prepare spinning solutions A and B

containing 23% of the polymer components A and B, respectively. The spinning solutions A and B were extruded from a spinneret in a conjugate ratio (weight ratio) of component A/component B of 5/5 and in a side-by-side relation into a coagulation bath consisting of a 56% DMF aqueous solution kept at 15° C. The extruded filaments were subjected to a primary drawing to draw the filaments to 4 times their original length. The primarily drawn filaments were washed with water, dried by means of a hot roller type drier kept at 125° C. until the water content of the filaments was decreased to 0.5%, and subjected to a secondary drawing at 115° C. under wet heat to draw the filaments to 1.3 times their original length, and the secondarily drawn filaments were subjected to a primary shrinking at 130° C. under wet heat to shrink the filaments to 0.9 time their original length.

Then, in order to improve the crimpability of the filaments, the above treated filaments were further subjected to a tertiary drawing at 180° C. under dry heat to draw the filaments to 1.4 times their original length, and the above drawn filaments were subjected to a secondary shrinking at 150° C. under dry heat to shrink the filaments to 0.9 times their original length. Then, the above treated filaments were mechanically crimped, and the crimps were set to obtain 3-denier composite fibers having a latent crimpability. The composite fiber obtained in the present invention has substantially the same crimpability as that of comparative sample and further has improved dyeability and water-absorbing property. Properties of the above obtained fibers are shown in the following Table 19.

TABLE 19

| Experiment number | Polymer component    |                          |                      | Fiber property       |            |              |                    |
|-------------------|----------------------|--------------------------|----------------------|----------------------|------------|--------------|--------------------|
|                   | Component A<br>x (%) | Component B<br>C (parts) | Component B<br>y (%) | Water absorption (%) | Dyeability | Crimpability | Remarks            |
| 213               | 7                    | 10                       | 9                    | 24                   | good       | good         | Present invention  |
| 214               | "                    | 20                       | "                    | 31                   | "          | "            | Present invention  |
| 215               | "                    | 30                       | "                    | 35                   | "          | "            | Present invention  |
| 216               | 10                   | 10                       | 8                    | 21                   | "          | "            | Present invention  |
| 217               | "                    | 20                       | "                    | 29                   | "          | "            | Present invention  |
| 218               | "                    | 30                       | "                    | 34                   | "          | "            | Present invention  |
| 219               | 7                    | 0                        | 9                    | 4                    | "          | "            | Comparative sample |
| 220               | 10                   | 0                        | 8                    | 4                    | "          | "            | Comparative sample |

EXAMPLE 21

A polymer component A consisting of 70 parts of an acrylic polymer, which had a composition of AN:MA:SMAS=91.5:8.0:0.5(%), 30 parts of cellulose acetate and 10 parts of an acrylic copolymer having a composition of  $\text{AN:CH}_2=\text{CHCOO}-\text{CH}_2\text{C}(\text{H}_2\text{O})_{20}\text{H}=90:10$ (%), and a component polymer B consisting of an acrylic polymer, which had a composition of AN:MA:SMAS=89.5:10.0:0.5(%), were separately dissolved in DMF to prepare spinning solutions A and B containing 23% of the polymer components A and B, respectively. The spinning solutions A and B were conjugate spun in a conjugate ratio (weight ratio) of component A/component B of 5/5. The spinning and the after-treatment were effected under the same spinning

and after-treatment conditions as described in Example 20 to obtain 3-denier composite fibers having a latent crimpability.

The resulting composite fiber had a porosity of 0.20 cm<sup>3</sup>/g, a surface area of voids of 1.13 m<sup>2</sup>/g and a water absorption of 27%. In the fiber, crimps were able to be easily developed by treating the fibers with boiling water at 100° C. for 5 minutes. The crimped fiber had a strength of 2.7 g/d, an elongation of 32.3%, a number of crimps of 32 per inch of fiber, a percentage crimp of 46%, an elastic recovery of crimp of 74% and a residual percentage crimp of 34%, and further had an excellent bulkiness.

## EXAMPLE 22

A polymer component A consisting of (100-C<sub>1</sub>) parts of an acrylic polymer, which had a composition of AN:MA:SMAS=92.4:7.0:0.6(%), and C<sub>1</sub> parts of cellulose acetate was dissolved in DMF to prepare a spinning solution A consisting of 23% of the polymer component A. A polymer component B consisting of (100-C<sub>2</sub>) parts of an acrylic polymer, which had a composition of AN:MA:SMAS=90.4:9.0:0.6(%), and C<sub>2</sub> parts of cellulose acetate was dissolved in DMF to prepare a spinning solution B containing 23% of the polymer component B. The spinning solutions A and B were extruded from a spinneret in a conjugate ratio of component A/component B of 1:1 and in a side-by-side relation into a coagulation bath consisting of a 56% DMF aqueous solution kept at 16° C. The extruded filaments were subjected to a primary drawing to draw the filaments to 4 times their original length, washed

with water and then dried by means of a hot roller type drier kept at 125° C. until the water content of the filaments was decreased to 0.7%. The dried filaments were subjected to a secondary drawing at 110° C. under wet heat to draw the filaments to 1.6 times their original length, the secondarily drawn filaments were subjected to a primary shrinking at 125° C. under wet heat to shrink the filaments to 0.9 time their original length, the primarily shrunk filaments were subjected to a tertiary drawing at 180° C. under dry heat to draw the filaments to 1.4 times their original length, and then the drawn filaments were subjected to a secondary shrinking at 150° C. under dry heat to shrink the filaments to 0.9 times their original length. The above treated filaments were mechanically crimped and the crimps were set to obtain composite fibers having a latent crimpability.

Properties of the composite fibers are shown in the following Table 20.

## EXAMPLE 23

TABLE 20(a)

| Experiment number | Polymer component         |                           | Void  | Fiber property                   |                                     |                      |                                             | Remarks            |
|-------------------|---------------------------|---------------------------|-------|----------------------------------|-------------------------------------|----------------------|---------------------------------------------|--------------------|
|                   | C <sub>1</sub><br>(parts) | C <sub>2</sub><br>(parts) |       | Porosity<br>(cm <sup>3</sup> /g) | Surface area<br>(m <sup>2</sup> /g) | Water absorption (%) | Dyeability                                  |                    |
| 221               | 2                         | 2                         | 0.105 | 1.35                             | 14                                  | good                 |                                             | Present invention  |
| 222               | "                         | 10                        | 0.231 | 1.62                             | 26                                  | "                    |                                             | Present invention  |
| 223               | "                         | 20                        | 0.294 | 1.84                             | 33                                  | "                    |                                             | Present invention  |
| 224               | "                         | 30                        | 0.357 | 2.01                             | 38                                  | "                    |                                             | Present invention  |
| 225               | "                         | 50                        | 0.731 | 2.56                             | 77                                  | somewhat poor        | somewhat poor in strength and in elongation | Present invention  |
| 226               | "                         | 60                        | 0.945 | 2.94                             | 94                                  | poor                 | poor in strength and in elongation          | Comparative sample |
| 227               | 10                        | 2                         | 0.245 | 1.43                             | 27                                  | good                 |                                             | Present invention  |
| 228               | "                         | 10                        | 0.357 | 1.76                             | 38                                  | "                    |                                             | Present invention  |
| 229               | "                         | 30                        | 0.483 | 1.89                             | 50                                  | "                    |                                             | Present invention  |

TABLE 20(b)

| Experiment number | Polymer component         |                           | Void  | Fiber property                   |                                     |                      |                                             | Remarks            |
|-------------------|---------------------------|---------------------------|-------|----------------------------------|-------------------------------------|----------------------|---------------------------------------------|--------------------|
|                   | C <sub>1</sub><br>(parts) | C <sub>2</sub><br>(parts) |       | Porosity<br>(cm <sup>3</sup> /g) | Surface area<br>(m <sup>2</sup> /g) | Water absorption (%) | Dyeability                                  |                    |
| 230               | 10                        | 50                        | 0.851 | 1.91                             | 84                                  | somewhat poor        | poor in strength and in elongation          | Comparative sample |
| 231               | 30                        | 10                        | 0.473 | 1.94                             | 49                                  | good                 |                                             | Present invention  |
| 232               | "                         | 30                        | 0.578 | 2.57                             | 60                                  | somewhat poor        | somewhat poor in strength and in elongation | Present invention  |
| 233               | "                         | 50                        | 0.945 | 3.48                             | 100                                 | poor                 | poor in strength and in elongation          | Comparative sample |
| 234               | 2                         | 10                        | 0.231 | 1.62                             | 25                                  | good                 |                                             | Present invention  |
| 235               | 10                        | "                         | 0.353 | 1.75                             | 39                                  | "                    |                                             | Present invention  |
| 236               | 30                        | "                         | 0.476 | 1.94                             | 51                                  | "                    |                                             | Present invention  |
| 237               | 50                        | "                         | 0.735 | 2.41                             | 74                                  | somewhat poor        | somewhat poor in strength and in elongation | Present invention  |

A polymer component A consisting of (100-C<sub>1</sub>) parts of an acrylic polymer, which had a composition of AN:MA:SMAS=92.4:7.0:0.6(%), and C<sub>1</sub> parts of cellu-

TABLE 20(c)

| Experiment number | Polymer component         |                           | Void  | Fiber property                   |                                     |                      |                                             | Remarks            |
|-------------------|---------------------------|---------------------------|-------|----------------------------------|-------------------------------------|----------------------|---------------------------------------------|--------------------|
|                   | C <sub>1</sub><br>(parts) | C <sub>2</sub><br>(parts) |       | Porosity<br>(cm <sup>3</sup> /g) | Surface area<br>(m <sup>2</sup> /g) | Water absorption (%) | Dyeability                                  |                    |
| 238               | 60                        | 10                        | 1.007 | 2.98                             | 117                                 | poor                 | poor in strength and in elongation          | Comparative sample |
| 239               | 2                         | 30                        | 0.315 | 1.88                             | 33                                  | good                 |                                             | Present invention  |
| 240               | 10                        | "                         | 0.469 | 1.93                             | 49                                  | "                    |                                             | Present invention  |
| 241               | 30                        | "                         | 0.563 | 2.57                             | 58                                  | somewhat poor        | somewhat poor in strength and in elongation | Present invention  |
| 242               | 50                        | "                         | 0.913 | 3.49                             | 92                                  | poor                 | poor in strength and in elongation          | Comparative sample |

lose acetate was dissolved in DMF to prepare a spinning solution A containing 23% of the polymer component A. A polymer component B consisting of (100-C<sub>2</sub>) parts of an acrylic copolymer, which had a composition of AN:MA:SMAS=89.4:10.0:0.6(%), and C<sub>2</sub> parts of cellulose acetate was dissolved in DMF to prepare a spinning solution B containing 23% of the polymer

solution kept at 16° C. The spinning, drawing and after-treatment were carried out under the same conditions as described in Example 22 to obtain 3-denier composite fibers having a latent crimpability. The fibers were treated in hot water kept at 100° C. for 5 minutes to develop crimps. Properties of the fibers are shown in Table 21.

TABLE 21 (a)

| Experiment number | Polymer component      |                        | Conjugate ratio A/B | Void Porosity (cm <sup>3</sup> /g) | Fiber property       |                       | Remarks            |
|-------------------|------------------------|------------------------|---------------------|------------------------------------|----------------------|-----------------------|--------------------|
|                   | C <sub>1</sub> (parts) | C <sub>2</sub> (parts) |                     |                                    | Water absorption (%) | Number of crimps/inch |                    |
| 243               | 2                      | 28                     | 8/2                 | 0.205                              | 23                   | 11                    | Comparative sample |
| 244               | "                      | "                      | 7/3                 | 0.221                              | 25                   | 23                    | Present invention  |
| 245               | "                      | "                      | 6/4                 | 0.293                              | 33                   | 44                    | Present invention  |
| 246               | "                      | "                      | 5/5                 | 0.339                              | 35                   | 52                    | Present invention  |
| 247               | "                      | "                      | 4/6                 | 0.374                              | 39                   | 48                    | Present invention  |
| 248               | "                      | "                      | 3/7                 | 0.416                              | 44                   | 29                    | Present invention  |
| 249               | "                      | "                      | 2/8                 | 0.473                              | 49                   | 13                    | Comparative sample |
| 250               | 7                      | 23                     | 8/2                 | 0.320                              | 35                   | 14                    | Comparative sample |
| 251               | "                      | "                      | 7/3                 | 0.343                              | 34                   | 25                    | Present invention  |
| 252               | "                      | "                      | 6/4                 | 0.364                              | 38                   | 48                    | Present invention  |
| 253               | "                      | "                      | 5/5                 | 0.381                              | 41                   | 61                    | Present invention  |
| 254               | "                      | "                      | 4/6                 | 0.409                              | 43                   | 50                    | Present invention  |
| 255               | "                      | "                      | 3/7                 | 0.429                              | 45                   | 31                    | Present invention  |

TABLE 21(b)

| Experiment Number | Polymer component      |                        | Conjugate ratio A/B | Void Porosity (cm <sup>3</sup> /g) | Fiber property       |                       | Remarks            |
|-------------------|------------------------|------------------------|---------------------|------------------------------------|----------------------|-----------------------|--------------------|
|                   | C <sub>1</sub> (parts) | C <sub>2</sub> (parts) |                     |                                    | Water absorption (%) | Number of crimps/inch |                    |
| 256               | 7                      | 23                     | 2/8                 | 0.453                              | 48                   | 17                    | Comparative sample |
| 257               | 15                     | 15                     | 8/2                 | 0.403                              | 41                   | 13                    | Comparative sample |
| 258               | "                      | "                      | 7/3                 | 0.414                              | 43                   | 25                    | Present invention  |
| 259               | "                      | "                      | 5/5                 | 0.404                              | 45                   | 54                    | Present invention  |
| 260               | "                      | "                      | 3/7                 | 0.407                              | 41                   | 29                    | Present invention  |
| 261               | "                      | "                      | 2/8                 | 0.409                              | 43                   | 16                    | Comparative sample |
| 262               | 10                     | 10                     | 8/2                 | 0.357                              | 37                   | 15                    | Comparative sample |
| 263               | "                      | "                      | 7/3                 | 0.363                              | 39                   | 26                    | Present invention  |
| 264               | "                      | "                      | 6/4                 | 0.351                              | 36                   | 47                    | Present invention  |
| 265               | "                      | "                      | 5/5                 | 0.349                              | 37                   | 58                    | Present invention  |
| 266               | "                      | "                      | 4/6                 | 0.353                              | 38                   | 51                    | Present invention  |
| 267               | "                      | "                      | 3/7                 | 0.364                              | 38                   | 34                    | Present invention  |
| 268               | "                      | "                      | 2/8                 | 0.358                              | 37                   | 17                    | Comparative sample |

component B. The spinning solutions A and B were extruded from a spinneret in various conjugate ratios (weight ratio of component A/component B) shown in the following Table 21 and in a side-by-side relation into a coagulation bath consisting of a 56% DMF aqueous

## EXAMPLE 24

A polymer component A consisting of 90 parts of an acrylic polymer, which had a composition of AN:(M-1):SMAS=(99.5-x):x:0.5(%), and 10 parts of cellulose

acetate, and a polymer component B consisting of 90 parts of an acrylic copolymer, which had a composition of AN:(M-2):SMAS=(99.5-y):y:0.5(%), and 10 parts of cellulose acetate were separately dissolved in DMF to prepare spinning solutions A and B containing 25% of the polymer components A and B, respectively. The spinning solutions A and B were extruded from a spinneret in a conjugate ratio (weight ratio of component A/component B) of 5/5 and in a side-by-side relation into a coagulation bath consisting of a 56% DMF aqueous solution kept at 20° C. The extruded filaments were

5 times their original length, washed with water, and then dried by means of a hot roller type drier kept at 125° C. until the water content of the filaments was decreased to not more than 0.7%. After the drying, the dried filaments were treated under the same conditions as described in Example 22 to obtain 3-denier composite fibers having a latent crimpability. The fibers were treated in hot water kept at 100° C. for 5 minutes to develop crimps.

Properties of the fibers are shown in the following Table 22.

TABLE 22(a)

| Experiment number | Polymer component |       |                 |       | Fiber property                     |                      |                       |              |                    |
|-------------------|-------------------|-------|-----------------|-------|------------------------------------|----------------------|-----------------------|--------------|--------------------|
|                   | Polymer A         |       | Polymer B       |       | Void Porosity (cm <sup>3</sup> /g) | Water absorption (%) | Number of crimps/inch | Crimpability | Remarks            |
|                   | M-1               | x (%) | M-2             | y (%) |                                    |                      |                       |              |                    |
| 269               | methyl acrylate   | 5     | methyl acrylate | 6     | 0.347                              | 36                   | 13                    | poor         | Comparative sample |
| 270               | "                 | "     | "               | 6.5   | 0.349                              | 37                   | 16                    | "            | Comparative sample |
| 271               | "                 | "     | "               | 7     | 0.351                              | 37                   | 34                    | high         | Present invention  |
| 272               | "                 | "     | "               | 7.5   | 0.356                              | 38                   | 47                    | "            | Present invention  |
| 273               | "                 | "     | "               | 8     | 0.371                              | 40                   | 53                    | "            | Present invention  |
| 274               | "                 | 6     | "               | 7     | 0.353                              | 36                   | 11                    | poor         | Comparative sample |
| 275               | "                 | "     | "               | 7.5   | 0.355                              | 37                   | 15                    | "            | Comparative sample |
| 276               | "                 | "     | "               | 8     | 0.361                              | 36                   | 28                    | high         | Present invention  |
| 277               | "                 | "     | "               | 8.5   | 0.367                              | 39                   | 39                    | "            | Present invention  |
| 278               | "                 | "     | "               | 9     | 0.371                              | 39                   | 47                    | "            | Present invention  |

TABLE 22(b)

| Experiment number | Polymer component |       |                 |       | Fiber property                     |                      |                       |              |                    |
|-------------------|-------------------|-------|-----------------|-------|------------------------------------|----------------------|-----------------------|--------------|--------------------|
|                   | Polymer A         |       | Polymer B       |       | Void Porosity (cm <sup>3</sup> /g) | Water absorption (%) | Number of crimps/inch | Crimpability | Remarks            |
|                   | M-1               | x (%) | M-2             | y (%) |                                    |                      |                       |              |                    |
| 279               | methyl acrylate   | 7     | methyl acrylate | 8     | 0.357                              | 38                   | 12                    | poor         | Comparative sample |
| 280               | "                 | "     | "               | 8.5   | 0.363                              | 38                   | 17                    | "            | Comparative sample |
| 281               | "                 | "     | "               | 9     | 0.361                              | 38                   | 31                    | high         | Present invention  |
| 282               | "                 | "     | "               | 9.5   | 0.371                              | 39                   | 43                    | "            | Present invention  |
| 283               | "                 | "     | "               | 10    | 0.365                              | 38                   | 54                    | "            | Present invention  |
| 284               | "                 | 9     | "               | 10.5  | 0.351                              | 37                   | 16                    | poor         | Comparative sample |
| 285               | "                 | "     | "               | 11    | 0.353                              | 37                   | 31                    | high         | Present invention  |
| 286               | "                 | "     | "               | 12    | 0.347                              | 36                   | 45                    | "            | Present invention  |

subjected to a primary drawing to draw the filaments to

TABLE 22(c)

| Experiment number | Polymer component |       |                 |       | Fiber property                     |                      |                       |              |                    |
|-------------------|-------------------|-------|-----------------|-------|------------------------------------|----------------------|-----------------------|--------------|--------------------|
|                   | Polymer A         |       | Polymer B       |       | Void Porosity (cm <sup>3</sup> /g) | Water absorption (%) | Number of crimps/inch | Crimpability | Remarks            |
|                   | M-1               | x (%) | M-2             | y (%) |                                    |                      |                       |              |                    |
| 287               | methyl acrylate   | 10    | methyl acrylate | 11.5  | 0.341                              | 36                   | 14                    | poor         | Comparative sample |
| 288               | "                 | "     | "               | 12    | 0.337                              | 35                   | 29                    | high         | Present invention  |
| 289               | "                 | "     | "               | 13    | 0.329                              | 34                   | 41                    | "            | Present            |

TABLE 22(c)-continued

| Experiment number | Polymer component |       |               |       | Void Porosity (cm <sup>3</sup> /g) | Fiber property         |                       |               |             |
|-------------------|-------------------|-------|---------------|-------|------------------------------------|------------------------|-----------------------|---------------|-------------|
|                   | Polymer A         |       | Polymer B     |       |                                    | Water absorp- tion (%) | Number of crimps/inch | Crimp-ability | Remarks     |
|                   | M-1               | x (%) | M-2           | y (%) |                                    |                        |                       |               |             |
| 290               | "                 | "     | "             | 14    | 0.325                              | 34                     | 56                    | "             | invention   |
| 291               | vinyl acetate     | 9.0   | vinyl acetate | 10    | 0.374                              | 39                     | 11                    | poor          | Present     |
| 292               | "                 | "     | "             | 10.5  | 0.377                              | 41                     | 17                    | "             | Comparative |
| 293               | "                 | "     | "             | 11.0  | 0.383                              | 40                     | 28                    | high          | sample      |
| 294               | "                 | "     | "             | 11.5  | 0.371                              | 39                     | 37                    | "             | Comparative |
| 295               | "                 | "     | "             | 12.0  | 0.363                              | 38                     | 49                    | "             | Present     |
| 296               | "                 | "     | "             | 12.5  | 0.358                              | 37                     | 56                    | "             | invention   |

TABLE 22(d)

| Experiment number | Polymer component                                                     |       |                                                                        |               | Void Porosity (cm <sup>3</sup> /g) | Fiber property         |                       |               |             |
|-------------------|-----------------------------------------------------------------------|-------|------------------------------------------------------------------------|---------------|------------------------------------|------------------------|-----------------------|---------------|-------------|
|                   | Polymer A                                                             |       | Polymer B                                                              |               |                                    | Water absorp- tion (%) | Number of crimps/inch | Crimp-ability | Remarks     |
|                   | M-1                                                                   | x (%) | M-2                                                                    | y (%)         |                                    |                        |                       |               |             |
| 297               | a mixture of<br>7% of methyl<br>acrylate and<br>1% of acryl-<br>amide | 8     | a mixture of<br>7% of methyl<br>acrylate and<br>1% of acryl-<br>amide* | 9<br>(2*)     | 0.293                              | 31                     | 12                    | poor          | Comparative |
| 298               | a mixture of<br>7% of methyl<br>acrylate and<br>1% of acryl-<br>amide | "     | a mixture of<br>7% of methyl<br>acrylate and<br>1% of acryl-<br>amide* | 9.5<br>(2.5)  | 0.279                              | 30                     | 19                    | "             | sample      |
| 299               | a mixture of<br>7% of methyl<br>acrylate and<br>1% of acryl-<br>amide | "     | a mixture of<br>7% of methyl<br>acrylate and<br>1% of acryl-<br>amide* | 10<br>(3.0)   | 0.237                              | 27                     | 31                    | high          | Comparative |
| 300               | a mixture of<br>7% of methyl<br>acrylate and<br>1% of acryl-<br>amide | "     | a mixture of<br>7% of methyl<br>acrylate and<br>1% of acryl-<br>amide* | 10.5<br>(3.5) | 0.231                              | 25                     | 43                    | "             | sample      |
| 301               | a mixture of<br>7% of methyl<br>acrylate and<br>1% of acryl-<br>amide | "     | a mixture of<br>7% of methyl<br>acrylate and<br>1% of acryl-<br>amide* | 11<br>(4.0)   | 0.245                              | 26                     | 51                    | "             | Present     |
| 302               | methyl acrylate                                                       | 7     | 2-hydroxyethyl<br>methacrylate                                         | 9             | 0.349                              | 37                     | 13                    | poor          | Present     |
| 303               | "                                                                     | "     | 2-hydroxyethyl<br>methacrylate                                         | 9.5           | 0.353                              | 38                     | 17                    | "             | invention   |
| 304               | "                                                                     | "     | 2-hydroxyethyl<br>methacrylate                                         | 10            | 0.358                              | 39                     | 28                    | high          | Comparative |
| 305               | "                                                                     | "     | 2-hydroxyethyl<br>methacrylate                                         | 11            | 0.361                              | 40                     | 41                    | "             | sample      |

## EXAMPLE 25

60

A polymer component A consisting of 85 parts of an acrylic polymer, which had a composition of AN:MA:SMAS=9.06:9.0:0.4(%), and 15 parts of cellulose acetate, and a polymer component B consisting of 85 parts of an acrylic polymer, which had a composition of AN:MA:SMAS=87.5:12.0:0.5(%), and 15 parts of cellulose acetate were separately dissolved in DMF to prepare spinning solutions A and B containing 23% of

the polymer components A and B, respectively. The spinning solutions A and B were extruded from a spinneret in a conjugate ratio (weight ratio), of component A:component B of 5:5 and in a side-by-side relation into a coagulation bath consisting of a 65% DMF aqueous solution kept at 15° C. The extruded filaments were subjected to a primary drawing under the condition shown in the following Table 23, and washed with

water. Then, the filaments were dried and after-treated under the same conditions as described in Example 22 to obtain composite fibers having a latent crimpability. Properties of the fibers are shown in Table 23.

TABLE 23

| Experiment number | Draw ratio in primary drawing | Fiber property |                      |            |               |                                             |                                            | Remarks            |
|-------------------|-------------------------------|----------------|----------------------|------------|---------------|---------------------------------------------|--------------------------------------------|--------------------|
|                   |                               | Void           | Water absorption (%) | Dyeability | Others        | Operability                                 |                                            |                    |
| 306               | 2                             | 0.443          | 7.64                 | 43         | somewhat poor | somewhat poor in strength and in elongation | dried yarn is brittle                      | Comparative sample |
| 307               | 2.5                           | 0.435          | 4.35                 | 45         | somewhat poor | somewhat poor in strength and in elongation | dried yarn is brittle                      | Present invention  |
| 308               | 3                             | 0.432          | 2.31                 | 45         | good poor     | in strength and in elongation               | is brittle                                 | Present invention  |
| 309               | 4                             | 0.411          | 2.08                 | 43         | " poor        | in strength and in elongation               | is brittle                                 | Present invention  |
| 310               | 5                             | 0.403          | 2.11                 | 45         | " poor        | in strength and in elongation               | is brittle                                 | Present invention  |
| 311               | 6                             | 0.387          | 2.14                 | 39         | " poor        | in strength and in elongation               | is brittle                                 | Present invention  |
| 312               | 7                             | 0.374          | 2.31                 | 39         | " poor        | in strength and in elongation               | is brittle                                 | Present invention  |
| 313               | 8                             | 0.351          | 2.05                 | 37         | " poor        | in strength and in elongation               | is brittle                                 | Present invention  |
| 314               | 9                             | 0.330          | 1.88                 | 35         | "             |                                             | yarn breakage occurs often during spinning | Comparative sample |
| 315               | 10                            | 0.289          | 1.74                 | 31         | "             |                                             | yarn breakage occurs often during spinning | Comparative sample |

## EXAMPLE 26

The same spinning solutions A and B as described in Example 25 were extruded from a spinneret in a conjugate ratio of component A:component B of 5:5 and in a side-by-side relation into a coagulation bath consisting of a 65% DMF aqueous solution kept at 15° C. The

extruded filaments were subjected to a primary drawing to draw the filaments to 5 times their original length, washed with water and then dried at a drying temperature shown in the following Table 24 until the water

content of the filaments was decreased to not more than 0.7%. The dried filaments were subjected to a secondary drawing and the successive after-treatments under the same conditions as described in Example 22 to obtain 3-denier composite fibers having a latent crimpability. Properties of the fibers are shown in Table 24.

TABLE 24

| Experiment number | Drying temperature (°C.) | Fiber property |                      |            |               |                                             |  | Remarks            |
|-------------------|--------------------------|----------------|----------------------|------------|---------------|---------------------------------------------|--|--------------------|
|                   |                          | Void           | Water absorption (%) | Dyeability | Others        |                                             |  |                    |
| 316               | 60                       | 0.609          | 17.1                 | 56         | poor          | fiber is whitened and yarn property is poor |  | Comparative sample |
| 317               | 80                       | 0.537          | 16.3                 | 50         | "             | fiber is whitened and yarn property is poor |  | Comparative sample |
| 318               | 100                      | 0.411          | 6.55                 | 43         | somewhat poor |                                             |  | Present invention  |
| 319               | 120                      | 0.403          | 2.11                 | 45         | good          |                                             |  | Present invention  |
| 320               | 140                      | 0.389          | 1.74                 | 42         | "             |                                             |  | Present invention  |
| 321               | 160                      | 0.381          | 1.57                 | 41         | "             |                                             |  | Present invention  |
| 322               | 180                      | 0.368          | 1.35                 | 39         | "             |                                             |  | Present invention  |
| 323               | 190                      | 0.346          | 1.38                 | 37         | "             | fiber is colored                            |  | Comparative        |

TABLE 24-continued

| Experiment number | Drying temperature (°C.) | Fiber property                |                                  |             |               |                                                          |                           |
|-------------------|--------------------------|-------------------------------|----------------------------------|-------------|---------------|----------------------------------------------------------|---------------------------|
|                   |                          | Void                          | Water                            | Dye-ability | Others        | Remarks                                                  |                           |
|                   |                          | Porosity (cm <sup>3</sup> /g) | Surface area (m <sup>2</sup> /g) |             |               |                                                          |                           |
| 324               | 200                      | 0.312                         | 1.19                             | 35          | somewhat poor | and becomes brittle fiber is colored and becomes brittle | sample Comparative sample |

## EXAMPLE 27

The same water-washed filament tows as those obtained in Example 26, which had been swollen with water, were dried by means of hot roller type drier kept at 120° C. until the water content of the tows was decreased to various water contents shown in the following Table 25, and the dried tows were treated under the same after-treatment conditions as described in Example 26 to obtain 3-denier composite fibers having a latent crimpability. Properties of the fibers are shown in Table 25.

15  
20  
25  
30  
35  
40  
45  
50  
55  
60  
65  
70  
75  
80  
85  
90  
95  
100  
105  
110  
115  
120  
125  
130  
135  
140  
145  
150  
155  
160  
165  
170  
175  
180  
185  
190  
195  
200  
205  
210  
215  
220  
225  
230  
235  
240  
245  
250  
255  
260  
265  
270  
275  
280  
285  
290  
295  
300  
305  
310  
315  
320  
325  
330  
335  
340  
345  
350  
355  
360  
365  
370  
375  
380  
385  
390  
395  
400  
405  
410  
415  
420  
425  
430  
435  
440  
445  
450  
455  
460  
465  
470  
475  
480  
485  
490  
495  
500  
505  
510  
515  
520  
525  
530  
535  
540  
545  
550  
555  
560  
565  
570  
575  
580  
585  
590  
595  
600  
605  
610  
615  
620  
625  
630  
635  
640  
645  
650  
655  
660  
665  
670  
675  
680  
685  
690  
695  
700  
705  
710  
715  
720  
725  
730  
735  
740  
745  
750  
755  
760  
765  
770  
775  
780  
785  
790  
795  
800  
805  
810  
815  
820  
825  
830  
835  
840  
845  
850  
855  
860  
865  
870  
875  
880  
885  
890  
895  
900  
905  
910  
915  
920  
925  
930  
935  
940  
945  
950  
955  
960  
965  
970  
975  
980  
985  
990  
995  
1000  
1005  
1010  
1015  
1020  
1025  
1030  
1035  
1040  
1045  
1050  
1055  
1060  
1065  
1070  
1075  
1080  
1085  
1090  
1095  
1100  
1105  
1110  
1115  
1120  
1125  
1130  
1135  
1140  
1145  
1150  
1155  
1160  
1165  
1170  
1175  
1180  
1185  
1190  
1195  
1200  
1205  
1210  
1215  
1220  
1225  
1230  
1235  
1240  
1245  
1250  
1255  
1260  
1265  
1270  
1275  
1280  
1285  
1290  
1295  
1300  
1305  
1310  
1315  
1320  
1325  
1330  
1335  
1340  
1345  
1350  
1355  
1360  
1365  
1370  
1375  
1380  
1385  
1390  
1395  
1400  
1405  
1410  
1415  
1420  
1425  
1430  
1435  
1440  
1445  
1450  
1455  
1460  
1465  
1470  
1475  
1480  
1485  
1490  
1495  
1500  
1505  
1510  
1515  
1520  
1525  
1530  
1535  
1540  
1545  
1550  
1555  
1560  
1565  
1570  
1575  
1580  
1585  
1590  
1595  
1600  
1605  
1610  
1615  
1620  
1625  
1630  
1635  
1640  
1645  
1650  
1655  
1660  
1665  
1670  
1675  
1680  
1685  
1690  
1695  
1700  
1705  
1710  
1715  
1720  
1725  
1730  
1735  
1740  
1745  
1750  
1755  
1760  
1765  
1770  
1775  
1780  
1785  
1790  
1795  
1800  
1805  
1810  
1815  
1820  
1825  
1830  
1835  
1840  
1845  
1850  
1855  
1860  
1865  
1870  
1875  
1880  
1885  
1890  
1895  
1900  
1905  
1910  
1915  
1920  
1925  
1930  
1935  
1940  
1945  
1950  
1955  
1960  
1965  
1970  
1975  
1980  
1985  
1990  
1995  
2000  
2005  
2010  
2015  
2020  
2025  
2030  
2035  
2040  
2045  
2050  
2055  
2060  
2065  
2070  
2075  
2080  
2085  
2090  
2095  
2100  
2105  
2110  
2115  
2120  
2125  
2130  
2135  
2140  
2145  
2150  
2155  
2160  
2165  
2170  
2175  
2180  
2185  
2190  
2195  
2200  
2205  
2210  
2215  
2220  
2225  
2230  
2235  
2240  
2245  
2250  
2255  
2260  
2265  
2270  
2275  
2280  
2285  
2290  
2295  
2300  
2305  
2310  
2315  
2320  
2325  
2330  
2335  
2340  
2345  
2350  
2355  
2360  
2365  
2370  
2375  
2380  
2385  
2390  
2395  
2400  
2405  
2410  
2415  
2420  
2425  
2430  
2435  
2440  
2445  
2450  
2455  
2460  
2465  
2470  
2475  
2480  
2485  
2490  
2495  
2500  
2505  
2510  
2515  
2520  
2525  
2530  
2535  
2540  
2545  
2550  
2555  
2560  
2565  
2570  
2575  
2580  
2585  
2590  
2595  
2600  
2605  
2610  
2615  
2620  
2625  
2630  
2635  
2640  
2645  
2650  
2655  
2660  
2665  
2670  
2675  
2680  
2685  
2690  
2695  
2700  
2705  
2710  
2715  
2720  
2725  
2730  
2735  
2740  
2745  
2750  
2755  
2760  
2765  
2770  
2775  
2780  
2785  
2790  
2795  
2800  
2805  
2810  
2815  
2820  
2825  
2830  
2835  
2840  
2845  
2850  
2855  
2860  
2865  
2870  
2875  
2880  
2885  
2890  
2895  
2900  
2905  
2910  
2915  
2920  
2925  
2930  
2935  
2940  
2945  
2950  
2955  
2960  
2965  
2970  
2975  
2980  
2985  
2990  
2995  
3000  
3005  
3010  
3015  
3020  
3025  
3030  
3035  
3040  
3045  
3050  
3055  
3060  
3065  
3070  
3075  
3080  
3085  
3090  
3095  
3100  
3105  
3110  
3115  
3120  
3125  
3130  
3135  
3140  
3145  
3150  
3155  
3160  
3165  
3170  
3175  
3180  
3185  
3190  
3195  
3200  
3205  
3210  
3215  
3220  
3225  
3230  
3235  
3240  
3245  
3250  
3255  
3260  
3265  
3270  
3275  
3280  
3285  
3290  
3295  
3300  
3305  
3310  
3315  
3320  
3325  
3330  
3335  
3340  
3345  
3350  
3355  
3360  
3365  
3370  
3375  
3380  
3385  
3390  
3395  
3400  
3405  
3410  
3415  
3420  
3425  
3430  
3435  
3440  
3445  
3450  
3455  
3460  
3465  
3470  
3475  
3480  
3485  
3490  
3495  
3500  
3505  
3510  
3515  
3520  
3525  
3530  
3535  
3540  
3545  
3550  
3555  
3560  
3565  
3570  
3575  
3580  
3585  
3590  
3595  
3600  
3605  
3610  
3615  
3620  
3625  
3630  
3635  
3640  
3645  
3650  
3655  
3660  
3665  
3670  
3675  
3680  
3685  
3690  
3695  
3700  
3705  
3710  
3715  
3720  
3725  
3730  
3735  
3740  
3745  
3750  
3755  
3760  
3765  
3770  
3775  
3780  
3785  
3790  
3795  
3800  
3805  
3810  
3815  
3820  
3825  
3830  
3835  
3840  
3845  
3850  
3855  
3860  
3865  
3870  
3875  
3880  
3885  
3890  
3895  
3900  
3905  
3910  
3915  
3920  
3925  
3930  
3935  
3940  
3945  
3950  
3955  
3960  
3965  
3970  
3975  
3980  
3985  
3990  
3995  
4000  
4005  
4010  
4015  
4020  
4025  
4030  
4035  
4040  
4045  
4050  
4055  
4060  
4065  
4070  
4075  
4080  
4085  
4090  
4095  
4100  
4105  
4110  
4115  
4120  
4125  
4130  
4135  
4140  
4145  
4150  
4155  
4160  
4165  
4170  
4175  
4180  
4185  
4190  
4195  
4200  
4205  
4210  
4215  
4220  
4225  
4230  
4235  
4240  
4245  
4250  
4255  
4260  
4265  
4270  
4275  
4280  
4285  
4290  
4295  
4300  
4305  
4310  
4315  
4320  
4325  
4330  
4335  
4340  
4345  
4350  
4355  
4360  
4365  
4370  
4375  
4380  
4385  
4390  
4395  
4400  
4405  
4410  
4415  
4420  
4425  
4430  
4435  
4440  
4445  
4450  
4455  
4460  
4465  
4470  
4475  
4480  
4485  
4490  
4495  
4500  
4505  
4510  
4515  
4520  
4525  
4530  
4535  
4540  
4545  
4550  
4555  
4560  
4565  
4570  
4575  
4580  
4585  
4590  
4595  
4600  
4605  
4610  
4615  
4620  
4625  
4630  
4635  
4640  
4645  
4650  
4655  
4660  
4665  
4670  
4675  
4680  
4685  
4690  
4695  
4700  
4705  
4710  
4715  
4720  
4725  
4730  
4735  
4740  
4745  
4750  
4755  
4760  
4765  
4770  
4775  
4780  
4785  
4790  
4795  
4800  
4805  
4810  
4815  
4820  
4825  
4830  
4835  
4840  
4845  
4850  
4855  
4860  
4865  
4870  
4875  
4880  
4885  
4890  
4895  
4900  
4905  
4910  
4915  
4920  
4925  
4930  
4935  
4940  
4945  
4950  
4955  
4960  
4965  
4970  
4975  
4980  
4985  
4990  
4995  
5000  
5005  
5010  
5015  
5020  
5025  
5030  
5035  
5040  
5045  
5050  
5055  
5060  
5065  
5070  
5075  
5080  
5085  
5090  
5095  
5100  
5105  
5110  
5115  
5120  
5125  
5130  
5135  
5140  
5145  
5150  
5155  
5160  
5165  
5170  
5175  
5180  
5185  
5190  
5195  
5200  
5205  
5210  
5215  
5220  
5225  
5230  
5235  
5240  
5245  
5250  
5255  
5260  
5265  
5270  
5275  
5280  
5285  
5290  
5295  
5300  
5305  
5310  
5315  
5320  
5325  
5330  
5335  
5340  
5345  
5350  
5355  
5360  
5365  
5370  
5375  
5380  
5385  
5390  
5395  
5400  
5405  
5410  
5415  
5420  
5425  
5430  
5435  
5440  
5445  
5450  
5455  
5460  
5465  
5470  
5475  
5480  
5485  
5490  
5495  
5500  
5505  
5510  
5515  
5520  
5525  
5530  
5535  
5540  
5545  
5550  
5555  
5560  
5565  
5570  
5575  
5580  
5585  
5590  
5595  
5600  
5605  
5610  
5615  
5620  
5625  
5630  
5635  
5640  
5645  
5650  
5655  
5660  
5665  
5670  
5675  
5680  
5685  
5690  
5695  
5700  
5705  
5710  
5715  
5720  
5725  
5730  
5735  
5740  
5745  
5750  
5755  
5760  
5765  
5770  
5775  
5780  
5785  
5790  
5795  
5800  
5805  
5810  
5815  
5820  
5825  
5830  
5835  
5840  
5845  
5850  
5855  
5860  
5865  
5870  
5875  
5880  
5885  
5890  
5895  
5900  
5905  
5910  
5915  
5920  
5925  
5930  
5935  
5940  
5945  
5950  
5955  
5960  
5965  
5970  
5975  
5980  
5985  
5990  
5995  
6000  
6005  
6010  
6015  
6020  
6025  
6030  
6035  
6040  
6045  
6050  
6055  
6060  
6065  
6070  
6075  
6080  
6085  
6090  
6095  
6100  
6105  
6110  
6115  
6120  
6125  
6130  
6135  
6140  
6145  
6150  
6155  
6160  
6165  
6170  
6175  
6180  
6185  
6190  
6195  
6200  
6205  
6210  
6215  
6220  
6225  
6230  
6235  
6240  
6245  
6250  
6255  
6260  
6265  
6270  
6275  
6280  
6285  
6290  
6295  
6300  
6305  
6310  
6315  
6320  
6325  
6330  
6335  
6340  
6345  
6350  
6355  
6360  
6365  
6370  
6375  
6380  
6385  
6390  
6395  
6400  
6405  
6410  
6415  
6420  
6425  
6430  
6435  
6440  
6445  
6450  
6455  
6460  
6465  
6470  
6475  
6480  
6485  
6490  
6495  
6500  
6505  
6510  
6515  
6520  
6525  
6530  
6535  
6540  
6545  
6550  
6555  
6560  
6565  
6570  
6575  
6580  
6585  
6590  
6595  
6600  
6605  
6610  
6615  
6620  
6625  
6630  
6635  
6640  
6645  
6650  
6655  
6660  
6665  
6670  
6675  
6680  
6685  
6690  
6695  
6700  
6705  
6710  
6715  
6720  
6725  
6730  
6735  
6740  
6745  
6750  
6755  
6760  
6765  
6770  
6775  
6780  
6785  
6790  
6795  
6800  
6805  
6810  
6815  
6820  
6825  
6830  
6835  
6840  
6845  
6850  
6855  
6860  
6865  
6870  
6875  
6880  
6885  
6890  
6895  
6900  
6905  
6910  
6915  
6920  
6925  
6930  
6935  
6940  
6945  
6950  
6955  
6960  
6965  
6970  
6975  
6980  
6985  
6990  
6995  
7000  
7005  
7010  
7015  
7020  
7025  
7030  
7035  
7040  
7045  
7050  
7055  
7060  
7065  
7070  
7075  
7080  
7085  
7090  
7095  
7100  
7105  
7110  
7115  
7120  
7125  
7130  
7135  
7140  
7145  
7150  
7155  
7160  
7165  
7170  
7175  
7180  
7185  
7190  
7195  
7200  
7205  
7210  
7215  
7220  
7225  
7230  
7235  
7240  
7245  
7250  
7255  
7260  
7265  
7270  
7275  
7280  
7285  
7290  
7295  
7300  
7305  
7310  
7315  
7320  
7325  
7330  
7335  
7340  
7345  
7350  
7355  
7360  
7365  
7370  
7375  
7380  
7385  
7390  
7395  
7400  
7405  
7410  
7415  
7420  
7425  
7430  
7435  
7440  
7445  
7450  
7455  
7460  
7465  
7470  
7475  
7480  
7485  
7490  
7495  
7500  
7505  
7510  
7515  
7520  
7525  
7530  
7535  
7540  
7545  
7550  
7555  
7560  
7565  
7570  
7575  
7580  
7585  
7590  
7595  
7600  
7605  
7610  
7615  
7620  
7625  
7630  
7635  
7640  
7645  
7650  
7655  
7660  
7665  
7670  
7675  
7680  
7685  
7690  
7695  
7700  
7705  
7710  
7715  
7720  
7725  
7730  
7735  
7740  
7745  
7750  
7755  
7760  
7765  
7770  
7775  
7780  
7785  
7790  
7795  
7800  
7805  
7810  
7815  
7820  
7825  
7830  
7835  
7840  
7845  
7850  
7855  
7860  
7865  
7870  
7875  
7880  
7885  
7890  
7895  
7900  
7905  
7910  
7915  
7920  
7925  
7930  
7935  
7940  
7945  
7950  
7955  
7960  
7965  
7970  
7975  
7980  
7985  
7990  
7995  
8000  
8005  
8010  
8015  
8020  
8025  
8030  
8035  
8040  
8045  
8050  
8055  
8060  
8065  
8070  
8075  
8080  
8085  
8090  
8095  
8100  
8105  
8110  
8115  
8120  
8125  
8130  
8135  
8140  
8145  
8150  
8155  
8160  
8165  
8170  
8175  
8180  
8185  
8190  
8195  
8200  
8205  
8210  
8215  
8220  
8225  
8230  
8235  
8240  
8245  
8250  
8255  
8260  
8265  
8270  
8275  
8280  
8285  
8290  
8295  
8300  
8305  
8310  
8315  
8320  
8325  
8330  
8335  
8340  
8345  
8350  
8355  
8360  
8365  
8370  
8375  
8380  
8385  
8390  
8395  
8400  
8405  
8410  
8415  
8420  
8425  
8430  
8435  
8440  
8445  
8450  
8455  
8460  
8465  
8470  
8475  
8480  
8485  
8490  
8495  
8500  
8505  
8510  
8515  
8520  
8525  
8530  
8535  
8540  
8545  
8550  
8555  
8560  
8565  
8570  
8575  
8580  
8585  
8590  
8595  
8600  
8605  
8610  
8615  
8620  
8625  
8630  
8635  
8640  
8645  
8650  
8655  
8660  
8665  
8670  
8675  
8680  
8685  
8690  
8695  
8700  
8705  
8710  
8715  
8720  
8725  
8730  
8735  
8740  
8745  
8750  
8755  
8760  
8765  
8770  
8775  
8780  
8785  
8790  
8795  
8800  
8805  
8810  
8815  
8820  
8825  
8830  
8835  
8840  
8845<br

TABLE 26

| Ex-<br>peri-<br>ment<br>num-<br>ber | Comonomer<br>in acrylic<br>copolymer (cm <sup>3</sup> /<br>g) | Before crimping       |                      |                          |                |                                   |                          | After crimping        |                      |                          |                       |                               |                                    | Residu-<br>al per-<br>cent-<br>age |    |    |
|-------------------------------------|---------------------------------------------------------------|-----------------------|----------------------|--------------------------|----------------|-----------------------------------|--------------------------|-----------------------|----------------------|--------------------------|-----------------------|-------------------------------|------------------------------------|------------------------------------|----|----|
|                                     |                                                               | Void                  |                      |                          | Fiber property |                                   |                          | Void                  |                      |                          | Fiber property        |                               |                                    |                                    |    |    |
|                                     |                                                               | Poros-<br>ity<br>area | Sur-<br>face<br>area | Water<br>absorp-<br>tion | Strength       | Elon-<br>(cm <sup>3</sup> /<br>g) | Water<br>absorp-<br>tion | Poros-<br>ity<br>area | Sur-<br>face<br>area | Water<br>absorp-<br>tion | Number<br>of<br>crimp | Per-<br>cent-<br>age<br>crimp | Elastic<br>recovery<br>of<br>crimp |                                    |    |    |
| R <sub>1</sub>                      | R <sub>2</sub>                                                | 1                     | m                    | (m <sup>2</sup> /g)      | (%)            | (g/d)                             | (%)                      | g)                    | (m <sup>2</sup> /g)  | (%)                      | inch                  | (%)                           | (%)                                | (%)                                |    |    |
| 334                                 | H                                                             | H                     | 0                    | 0                        | 0.351          | 1.98                              | 37                       | 3.1                   | 39                   | 0.355                    | 2.13                  | 36                            | 50                                 | 52                                 | 56 | 29 |
| 335                                 | H                                                             | H                     | 10                   | 0                        | 0.338          | 1.83                              | 35                       | 3.2                   | 41                   | 0.341                    | 2.07                  | 36                            | 51                                 | 55                                 | 55 | 30 |
| 336                                 | H                                                             | H                     | 10                   | 10                       | 0.335          | 2.01                              | 35                       | 3.0                   | 40                   | 0.339                    | 2.15                  | 35                            | 48                                 | 50                                 | 66 | 33 |
| 337                                 | CH <sub>3</sub>                                               | H                     | 15                   | 10                       | 0.364          | 2.15                              | 39                       | 3.2                   | 38                   | 0.368                    | 2.19                  | 38                            | 53                                 | 57                                 | 62 | 35 |
| 338                                 | CH <sub>3</sub>                                               | CH <sub>3</sub>       | 15                   | 20                       | 0.657          | 2.07                              | 37                       | 3.1                   | 39                   | 0.362                    | 2.24                  | 30                            | 55                                 | 59                                 | 63 | 37 |

What is claimed is:

1. Acrylic composite fibers having water absorption property wherein a component A consisting of 2~50% by weight of cellulose acetate and 50~98% by weight of an acrylic polymer and a component B consisting of an acrylic polymer are bonded in a conjugate ratio of 2/8~8/2 (by weight) along the fiber axial direction, the component A has substantially no microvoid but has mainly macrovoids, a porosity in the entire fibers is 25 0.05~0.75 cm<sup>3</sup>/g, a surface area of the voids is no greater than 15 m<sup>2</sup>/g, and the cellulose acetate is distributed in elongated forms along the axial directions of the fibers.

2. The fibers as claimed in claim 1, wherein the conjugate ratio of the component A and the component B is 30 3/7~7/3.

3. The fibers as claimed in claim 1, wherein the component A and the component B have difference in the shrinkability and are bonded eccentrically along the 35 fiber axial direction and said fibers have substantially latent crimpability.

4. The fibers as claimed in claim 1, wherein the component A and the component B have substantially no difference in the shrinkability and said fibers have no 40 latent crimpability.

5. Acrylic composite fibers having water absorption property and latent crimpability wherein two components A and B, consisting of 2~50% by weight of cellulose acetate and 50~98% by weight of an acrylic polymer and having difference of at least 2% by weight in a plasticizing component in the acrylic polymer, are bonded eccentrically in a conjugate ratio of 7/3~3/7 (by weight), said fibers have substantially no microvoids but mainly macrovoids, a porosity of 50 0.05~0.75 cm<sup>3</sup>/g and a surface area of voids no greater

than 15 m<sup>2</sup>/g, and the total amount of cellulose acetate in the fibers is 2~30% by weight which is distributed in elongated forms along the axial directions of said fibers.

6. The fibers as claimed in claim 5, wherein the plasticizing component is at least one of the group consisting of methyl acrylate, ethyl acrylate, methyl methacrylate, ethylmethacrylate, 2-hydroxyethyl acrylate, 2-hydroxyethyl methacrylate, acrylamide, methacrylamide and vinyl acetate.

7. The fibers as claimed in claim 1 or 5, wherein the acrylic polymer containing cellulose acetate contains 5~30% by weight of a monomer having the general formula



wherein X is R<sub>2</sub> or



R<sub>1</sub> and R<sub>3</sub> are H or CH<sub>3</sub>, R<sub>2</sub> is H, NH<sub>4</sub> or an alkali metal, and 1 and m are an integer of 0~50 and 0<1+m≤50, said acrylic copolymer being no greater than about 33% by weight based on the total polymer composing the acrylic composite fibers.

8. The fibers as claimed in claim 1 or 5, wherein the acrylic polymer contains at least 80% by weight of acrylonitrile and 0.3~1.5% by weight of a copolymerizable monomer containing sulfonic acid group.

\* \* \* \* \*